



US007169543B2

(12) **United States Patent**  
Ramsden et al.

(10) **Patent No.:** US 7,169,543 B2  
(45) **Date of Patent:** Jan. 30, 2007

|      |                                                                                                                                                                                                                                                                                                                                                                                |                   |         |                               |
|------|--------------------------------------------------------------------------------------------------------------------------------------------------------------------------------------------------------------------------------------------------------------------------------------------------------------------------------------------------------------------------------|-------------------|---------|-------------------------------|
| (54) | <b>BLOCKED ALIPHATIC THIOL STABILIZERS FOR PHOTOTHERMOGRAPHIC MATERIALS</b>                                                                                                                                                                                                                                                                                                    | 3,824,103 A       | 7/1974  | Pierce et al.                 |
| (75) | Inventors: <b>William D. Ramsden</b> , Afton, MN (US); <b>James B. Philip, Jr.</b> , Mahtomedi, MN (US); <b>Doreen C. Lynch</b> , Afton, MN (US); <b>Kui Chen-Ho</b> , Woodbury, MN (US); <b>Stacy M. Ulrich</b> , Dresser, WI (US); <b>Kumars Sakizadeh</b> , Woodbury, MN (US); <b>Jeffrey W. Leon</b> , Rochester, NY (US); <b>George J. Burgmaier</b> , Pittsford, NY (US) | 3,839,041 A       | 10/1974 | Hiller                        |
|      |                                                                                                                                                                                                                                                                                                                                                                                | 4,082,555 A       | 4/1978  | Merkel                        |
|      |                                                                                                                                                                                                                                                                                                                                                                                | 4,088,496 A       | 5/1978  | Merkel                        |
|      |                                                                                                                                                                                                                                                                                                                                                                                | 4,772,544 A       | 9/1988  | Hirai                         |
|      |                                                                                                                                                                                                                                                                                                                                                                                | 4,775,610 A       | 10/1988 | Kitaguchi et al.              |
|      |                                                                                                                                                                                                                                                                                                                                                                                | 4,983,494 A       | 1/1991  | Kitaguchi et al.              |
|      |                                                                                                                                                                                                                                                                                                                                                                                | 5,232,818 A *     | 8/1993  | Machonkin et al. .... 430/264 |
|      |                                                                                                                                                                                                                                                                                                                                                                                | 6,083,681 A       | 7/2000  | Lynch et al.                  |
|      |                                                                                                                                                                                                                                                                                                                                                                                | 6,379,880 B1      | 4/2002  | Katoh                         |
|      |                                                                                                                                                                                                                                                                                                                                                                                | 6,675,706 B2      | 1/2003  | Barker et al.                 |
|      |                                                                                                                                                                                                                                                                                                                                                                                | 6,558,896 B2      | 5/2003  | Komatsu                       |
|      |                                                                                                                                                                                                                                                                                                                                                                                | 6,605,418 B1      | 8/2003  | Ramsden et al.                |
|      |                                                                                                                                                                                                                                                                                                                                                                                | 6,737,277 B1      | 5/2004  | Kang et al.                   |
|      |                                                                                                                                                                                                                                                                                                                                                                                | 6,964,842 B2 *    | 11/2005 | Zou et al. .... 430/619       |
|      |                                                                                                                                                                                                                                                                                                                                                                                | 2002/0177090 A1   | 11/2002 | Ishihara                      |
|      |                                                                                                                                                                                                                                                                                                                                                                                | 2004/0126717 A1 * | 7/2004  | Nakagawa et al. .... 430/523  |

(73) Assignee: **Eastman Kodak Company**, Rochester, NY (US)

(\*) Notice: Subject to any disclaimer, the term of this patent is extended or adjusted under 35 U.S.C. 154(b) by 49 days.

(21) Appl. No.: 11/025,633

(22) Filed: Dec. 29, 2004

(65) **Prior Publication Data**

US 2006/0141403 A1 Jun. 29, 2006

(51) **Int. Cl.**

**G03C 5/16** (2006.01)  
**G03C 1/498** (2006.01)  
**G03C 1/34** (2006.01)

(52) **U.S. Cl.** .... **430/350**; 139/529; 139/600; 139/603; 139/611; 139/619; 139/955; 139/958; 430/966

(58) **Field of Classification Search** .... 430/619, 430/611, 955, 958, 959, 529, 600, 603, 629, 430/350, 139, 966

See application file for complete search history.

(56) **References Cited**

U.S. PATENT DOCUMENTS

3,301,678 A 1/1967 Humphlett et al.  
3,506,444 A 4/1970 Haist et al.  
3,531,285 A 9/1970 Haist et al.

|    |              |         |
|----|--------------|---------|
| DE | 33 16 985    | 5/1983  |
| EP | 0 863 432 A1 | 9/1998  |
| EP | 1 315 032    | 5/2003  |
| EP | 1 422 552    | 5/2004  |
| JP | 61-269147    | 11/1986 |
| JP | 2001-013617  | 1/2001  |
| JP | 2001-264932  | 9/2001  |
| JP | 2002-268180  | 9/2002  |

FOREIGN PATENT DOCUMENTS

|    |                       |
|----|-----------------------|
| JP | Abstract 01-167750.   |
| JP | Abstract 10-104782.   |
| JP | Abstract 2000-338624. |
| JP | Abstract 2001-056527. |
| *  | cited by examiner     |

Primary Examiner—Thorl Chea

(74) Attorney, Agent, or Firm—J. Lanny Tucker; Louis M. Leichter

(57) **ABSTRACT**

Photothermographic materials contain one or more blocked aliphatic thiol compounds in an amount of at least 1 mg/m<sup>2</sup> as stabilizers. These compounds have a calculated octanol-water partition coefficient (c log P value) of 2.0 or greater, and an N value equal to or greater than 6.5.

21 Claims, No Drawings

**BLOCKED ALIPHATIC THIOL  
STABILIZERS FOR  
PHOTOTHERMOGRAPHIC MATERIALS**

**FIELD OF THE INVENTION**

This invention relates to imaging materials comprising certain blocked aliphatic thiol compounds. In particular the invention relates to photothermographic materials containing these blocked aliphatic thiol compounds and to methods of imaging these materials.

**BACKGROUND OF THE INVENTION**

Silver-containing photothermographic imaging materials (that is, photothermographic photosensitive imaging materials) that are imaged with actinic radiation and then developed using heat and without liquid processing have been known in the art for many years. Such materials are used in a recording process wherein an image is formed by image-wise exposure of the photothermographic material to specific electromagnetic radiation and developed by the use of thermal energy. These materials, also known as "dry silver" materials, generally comprise a support having coated thereon: (a) a photocatalyst (that is, a photosensitive compound such as silver halide) that upon such exposure provides a latent image in exposed grains that are capable of acting as a catalyst for the subsequent formation of a silver image in a development step, (b) a relatively or completely non-photosensitive source of reducible silver ions, (c) a reducing composition (usually including a developer) for the reducible silver ions, and (d) a hydrophilic or hydrophobic binder. The latent image is then developed by application of thermal energy.

In photothermographic materials, exposure of the photographic silver halide to light produces small clusters containing silver atoms ( $\text{Ag}^0$ ). The imagewise distribution of these clusters, known in the art as a latent image, is generally not visible by ordinary means. Thus, the photosensitive material must be further developed to produce a visible image by the reduction of silver ions that are in catalytic proximity to silver halide grains bearing the silver-containing clusters of the latent image. This produces a black-and-white image. The non-photosensitive silver source is catalytically reduced to form the visible black-and-white negative image while much of the silver halide, generally, remains as silver halide and is not reduced. In most instances, the source of reducible silver ions is an organic silver salt in which silver ions are complexed with organic silver coordinating ligands.

**Differences Between Photothermography and Photography**

The imaging arts have long recognized that the field of photothermography is clearly distinct from that of photography. Photothermographic materials differ significantly from conventional silver halide photographic materials that require processing with aqueous processing solutions.

In photothermographic imaging materials, a visible image is created by heat as a result of the reaction of a developer incorporated within the material. Heating at 50° C. or more is essential for this dry development. In contrast, conventional photographic imaging materials require processing in aqueous processing baths at more moderate temperatures (from 30° C. to 50° C.) to provide a visible image.

In photothermographic materials, only a small amount of silver halide is used to capture light and a non-photosensitive source of reducible silver ions (for example a silver

carboxylate or a silver benzotriazole) is used to generate the visible image using thermal development. Thus, the imaged photosensitive silver halide serves as a catalyst for the physical development process involving the non-photosensitive source of reducible silver ions and the incorporated reducing agent. In contrast, conventional wet-processed, black-and-white photographic materials use only one form of silver (that is, silver halide) that, upon chemical development, is itself at least partially converted into the silver image, or that upon physical development requires addition of an external silver source (or other reducible metal ions that form black images upon reduction to the corresponding metal). Thus, photothermographic materials require an amount of silver halide per unit area that is only a fraction of that used in conventional wet-processed photographic materials.

In photothermographic materials, all of the "chemistry" for imaging is incorporated within the material itself. For example, such materials include a developer (that is, a reducing agent for the reducible silver ions) while conventional photographic materials usually do not. Even in so-called "instant photography," the developer chemistry is physically separated from the photosensitive silver halide until development is desired. The incorporation of the developer into photothermographic materials can lead to increased formation of various types of "fog" or other undesirable sensitometric side effects. Therefore, much effort has gone into the preparation and manufacture of photothermographic materials to minimize these problems.

Moreover, in photothermographic materials, the unexposed silver halide generally remains intact after development and the material must be stabilized against further imaging and development. In contrast, silver halide is removed from conventional photographic materials after solution development to prevent further imaging (that is in the aqueous fixing step).

Because photothermographic materials require dry thermal processing, they present distinctly different problems and require different materials in manufacture and use, compared to conventional, wet-processed silver halide photographic materials. Additives that have one effect in conventional silver halide photographic materials may behave quite differently when incorporated in photothermographic materials where the chemistry is significantly more complex. The incorporation of such additives as, for example, stabilizers, antifoggants, speed enhancers, supersensitizers, and spectral and chemical sensitizers in conventional photographic materials is not predictive of whether such additives will prove beneficial or detrimental in photothermographic materials. For example, it is not uncommon for a photographic antifoggant useful in conventional photographic materials to cause various types of fog when incorporated into photothermographic materials, or for supersensitizers that are effective in photographic materials to be inactive in photothermographic materials.

These and other distinctions between photothermographic and photographic materials are described in *Imaging Processes and Materials* (Nebblette's Eighth Edition), noted above, *Unconventional Imaging Processes*, E. Brinckman et al. (Eds.), The Focal Press, London and New York, 1978, pp. 74-75, in Zou et al., *J. Imaging Sci. Technol.* 1996, 40, pp. 94-103, and in M. R. V. Sahyun, *J. Imaging Sci. Technol.* 1998, 42, 23.

**Problem to be Solved**

A challenge in photothermographic materials is the need to improve their stability to light exposure after imaging and

processing. Referred to as "Desktop Print Stability" the formation of additional image or "print-out" is usually most evident as an increase in  $D_{min}$ . This effect tends to be a problem especially under high humidity conditions.

U.S. Pat. No. 3,824,103 (Pierce et al.) describes the use of certain S-carbamoyl compounds as silver salt stabilizer precursors for photothermographic materials at a level of about 0.25 to about 20 moles per mole of photosensitive silver salt.

U.S. Pat. No. 3,506,444 (Haist et al.), U.S. Pat. No. 3,531,285 (Haist et al.) and U.S. Pat. No. 3,301,678 (Humphlett et al.) describe certain sulfur-containing compounds that break down or cleave at elevated temperatures to form a compound that combines with the silver halide in the unexposed and undeveloped areas of the emulsion to form a silver mercaptide that is more stable than the silver halide to light.

Japanese Kokai 61-269147 (Kitaguchi et al.) describes a heat-developable photographic element containing a base or base precursor and a photographic reagent capable of releasing a compound of the formula  $RSH$  [where  $R=$ alkyl, alkenyl, aryl] on reacting with a base. The requirement of a base or a base precursor adds complexity to the system and does not function well in an acidic photothermographic material.

Japanese Kokai 2002-268180 (Maeda et al.) describes a heat-developable photographic element comprising a compound represented by the formula (1)



(1)

where Lv is O, N, or S.

Japanese Kokai 2001-013617 (Nobuaki et al.) describes a photothermographic material comprising a compound represented by formula  $W_1-S-ArH_1$  where  $W_1$  is a variety of blocking groups and  $ArH_1$  is an aromatic hydrocarbon group or an heteroaromatic group.

Japanese Kokai 2001-264932 (Kyoko et al.) describes a photothermographic material comprising a compound that is a blocked aromatic or heteroaromatic antifogger or print-out stabilizer.

There remains a need to find and incorporate compounds into photothermographic materials that improve Desktop Print Stability without sacrificing photospeed and other sensitometric properties.

#### SUMMARY OF THE INVENTION

The present invention provides a black-and-white photothermographic material comprising a support and having thereon at least one photothermographic imaging layer comprising a polymer binder and in reactive association:

- a. a photosensitive silver halide,
- b. a non-photosensitive source of reducible silver ions,
- c. a reducing agent for the reducible silver ions, and
- d. at least 1  $mg/m^2$  of a blocked aliphatic thiol compound that has a calculated octanol-water partition coefficient ( $c \log P$  value) 2.0 or greater, and an N value equal to or greater than 6.5.

Preferred embodiments of this invention include a black-and-white photothermographic material comprising a sup-

port and having thereon at least one photothermographic imaging layer comprising a hydrophilic polymer binder or a water-dispersible polymer latex binder and in reactive association:

- a. a photosensitive silver halide present as ultrathin tabular grains,
- b. a non-photosensitive source of reducible silver ions that comprises an organic silver salt comprising a silver salt of a nitrogen-containing heterocyclic compound containing an imino group,
- c. a reducing agent for the reducible silver ions that is an ascorbic acid derivative,
- d. a blocked aliphatic thiol compound that is represented by one or more of the compounds having Structures PS-1 through PS-47 described below, the blocked aliphatic thiol compound being present in an amount of from about 5  $mg/m^2$  to about 500  $mg/m^2$ , and
- e. boric acid or a boric acid ester compound. This invention also provides a black-and-white photothermographic material comprising a support having on a frontside thereof,
- a) one or more frontside photothermographic imaging layers comprising a polymer binder and in reactive association, a photosensitive silver halide, a non-photosensitive source of reducible silver ions, and a reducing agent for the non-photosensitive source reducible silver ions,
- b) the material comprising on the backside of the support, one or more backside photothermographic imaging layers having the same or different composition as the frontside photothermographic imaging layers, and
- c) optionally, an outermost protective layer disposed over the one or more photothermographic imaging layers on either or both sides of the support,
- wherein the material comprises one or more of the same or different blocked aliphatic thiol compounds on both sides of the support, each of the blocked aliphatic thiol compounds being present in the same or different amount of at least 1  $mg/m^2$  on both sides of the support, the blocked aliphatic thiol compound having a calculated octanol-water partition coefficient ( $c \log P$  value) of 2.0 or greater, and an N value equal to or greater than 6.5.

This invention also provides a method of forming a visible image comprising:

- (A) imagewise exposing the photothermographic material to form a latent image,
- (B) simultaneously or sequentially, heating the exposed photothermographic material to develop the latent image into a visible image.

The photothermographic material can be arranged in association with one or more phosphor intensifying screens in an imaging assembly.

We have found that the blocked aliphatic thiol compounds described herein are useful in improving the Desktop Print Stability of photothermographic materials, particularly in a high humidity environment. The presence of boric acid or a boric acid ester with the blocked aliphatic thiol compound provides even further stabilization. These results are achieved without significant loss in desired sensitometric properties and without the presence of a base or base precursor.

#### DETAILED DESCRIPTION OF THE INVENTION

The photothermographic materials can be used in black-and-white photothermography and in electronically gener-

ated black-and-white hardcopy recording. They can be used in microfilm applications, in radiographic imaging (for example digital medical imaging), X-ray radiography, and in industrial radiography. Furthermore, in some embodiments, the absorbance of these materials between 350 and 450 nm is desirably low (less than 0.5), to permit their use in the graphic arts area (for example, imagesetting and phototype-setting), in the manufacture of printing plates, in contact printing, in duplicating ("duping"), and in proofing.

The photothermographic materials are particularly useful for medical imaging of human or animal subjects in response to visible or X-radiation for use in medical diagnosis. Such applications include, but are not limited to, thoracic imaging, mammography, dental imaging, orthopedic imaging, general medical radiography, therapeutic radiography, veterinary radiography, and autoradiography. When used with X-radiation, the photothermographic materials may be used in association with one or more phosphor intensifying screens, with phosphors incorporated within the photothermographic emulsion, or with a combination thereof.

The photothermographic materials can be made sensitive to radiation of any suitable wavelength. Thus, in some embodiments, the materials are sensitive at ultraviolet, visible, near infrared, or infrared wavelengths, of the electromagnetic spectrum. In these embodiments, the materials are preferably sensitive to radiation greater than 300 nm (such as sensitivity to, from about 300 nm to about 850 nm, preferably from about 300 to about 600 nm, and more preferably from about 300 to about 450 nm). In other embodiments they are sensitive to X-radiation. Increased sensitivity to X-radiation can be imparted through the use of phosphors.

The photothermographic materials are also useful for non-medical uses of visible or X-radiation (such as X-ray lithography and industrial radiography). In these and other imaging applications, it is particularly desirable that the photothermographic materials be "double-sided."

In some embodiments of the photothermographic materials, the components needed for imaging can be in one or more imaging or emulsion layers on one side ("frontside") of the support. The layer(s) that contain the photosensitive photocatalyst (such as a photosensitive silver halide) for photothermographic materials or the non-photosensitive source of reducible silver ions, or both, are referred to herein as the emulsion layer(s). In photothermographic materials, the photocatalyst and non-photosensitive source of reducible silver ions are in catalytic proximity and preferably are in the same emulsion layer.

Where the photothermographic materials contain imaging layers on one side of the support only, various non-imaging layers can also be disposed on the "backside" (non-emulsion or non-imaging side) of the materials, including, conductive layers, antihalation layer(s), protective layers, antistatic layers, and transport enabling layers.

In such instances, various non-imaging layers can also be disposed on the "frontside" or imaging or emulsion side of the support, including protective overcoat layers, primer layers, interlayers, opacifying layers, antistatic layers, antihalation layers, acutance layers, auxiliary layers, and other layers readily apparent to one skilled in the art.

For preferred embodiments, the photothermographic materials are "double-sided" and have the same or different emulsion coatings (or photothermographic imaging layers) on both sides of the support. Such constructions can also include one or more protective overcoat layers, primer layers, interlayers, antistatic layers, acutance layers, antihalation layers, auxiliary layers, and other layers readily apparent to one skilled in the art.

lation layers, auxiliary layers, conductive layers, and other layers readily apparent to one skilled in the art on either or both sides of support. Preferably, such photothermographic materials have essentially the same layers on each side of the support.

When the photothermographic materials are heat-developed as described below in a substantially water-free condition after, or simultaneously with, imagewise exposure, a silver image (preferably a black-and-white silver image) is obtained.

#### Definitions

As used herein:

In the descriptions of the photothermographic materials, "a" or "an" component refers to "at least one" of that component (for example, the blocked aliphatic thiol compounds).

Unless otherwise indicated, the terms "thermally developable materials," "photothermographic materials," and "imaging assemblies" are used herein in reference to embodiments of the present invention.

Heating in a substantially water-free condition as used herein, means heating at a temperature of from about 50° C. to about 250° C. with little more than ambient water vapor present. The term "substantially water-free condition" means that the reaction system is approximately in equilibrium with water in the air and water for inducing or promoting the reaction is not particularly or positively supplied from the exterior to the material. Such a condition is described in T. H. James, *The Theory of the Photographic Process*, Fourth Edition, Eastman Kodak Company, Rochester, N.Y., 1977, p. 374.

"Photothermographic material(s)" means a construction comprising at least one photothermographic emulsion layer or a photothermographic set of emulsion layers (wherein the photosensitive silver halide and the source of reducible silver ions, are in one layer and the other essential components or desirable additives are distributed, as desired, in the same layer or in an adjacent coated layer). These materials also include multilayer constructions in which one or more imaging components are in different layers, but are in "reactive association." For example, one layer can include the non-photosensitive source of reducible silver ions and another layer can include the reducing agent and/or photosensitive silver halide.

When used in photothermography, the term, "imagewise exposing" or "imagewise exposure" means that the material is imaged using any exposure means that provides a latent image using electromagnetic radiation. This includes, for example, by analog exposure where an image is formed by projection onto the photosensitive material as well as by digital exposure where the image is formed one pixel at a time such as by modulation of scanning laser radiation.

"Catalytic proximity" or "reactive association" means that the materials are in the same layer or in adjacent layers so that they readily come into contact with each other during thermal imaging and development.

"Emulsion layer," "imaging layer," or "photothermographic emulsion layer," means a layer of a photothermographic material that contains the photosensitive silver halide and/or non-photosensitive source of reducible silver ions. It can also mean a layer of the material that contains, in addition to the photosensitive silver halide and/or non-photosensitive source of reducible ions, additional essential components and/or desirable additives such as the reducing agent(s). In "single-sided" materials, these layers are usually on what is known as the "frontside" of the support.

The terms "double sided" and "dupliclized" are used to define photothermographic materials having one or more of the same or different photothermographic emulsion layers disposed on both sides (front and back) of the support. In double-sided materials the emulsion layers can be of the same or different chemical composition, thickness, or sensitometric properties.

In addition, "frontside" also generally means the side of a photothermographic material that is first exposed to imaging radiation, and "backside" generally refers to the opposite side of the photothermographic material.

"Photocatalyst" means a photosensitive compound such as silver halide that, upon exposure to radiation, provides a compound that is capable of acting as a catalyst for the subsequent development of the photothermographic material.

Many of the materials used herein are provided as a solution. The term "active ingredient" means the amount or the percentage of the desired material contained in a sample.

"Ultraviolet region of the spectrum" refers to that region of the spectrum less than or equal to 410 nm, and preferably from about 100 nm to about 410 nm, although parts of these ranges may be visible to the naked human eye. More preferably, the ultraviolet region of the spectrum is the region of from about 190 nm to about 405 nm. The near ultraviolet region of the spectrum refers to that region of from about 300 to about 400 nm.

"Visible region of the spectrum" refers to that region of the spectrum of from about 400 nm to about 700 nm.

"Short wavelength visible region of the spectrum" refers to that region of the spectrum of from about 400 nm to about 450 nm.

"Blue region of the spectrum" refers to that region of the spectrum of from about 400 nm to about 500 nm.

"Green region of the spectrum" refers to that region of the spectrum of from about 500 nm to about 600 nm.

"Red region of the spectrum" refers to that region of the spectrum of from about 600 nm to about 700 nm.

"Infrared region of the spectrum" refers to that region of the spectrum of from about 700 nm to about 1400 nm.

"Non-photosensitive" means not intentionally light sensitive.

"Transparent" means capable of transmitting visible light or imaging radiation without appreciable scattering or absorption.

The sensitometric terms "photospeed," "speed," or "photographic speed" (also known as sensitivity), absorbance, contrast,  $D_{min}$ , and  $D_{max}$  have conventional definitions known in the imaging arts. In photothermographic materials,  $D_{min}$  is considered herein as image density achieved when the photothermographic material is thermally developed without prior exposure to radiation. It is the average of eight lowest density values on the exposed side of the fiducial mark.

In photothermographic materials, the term  $D_{max}$  is the maximum image density achieved when the photothermographic material is exposed to a particular radiation source and a given amount of radiation energy and then thermally developed.

The terms "density," "optical density (OD)," and "image density" refer to the sensitometric term absorbance.

"Speed-2" is  $\log 1/E+4$  corresponding to the density value of 1.0 above  $D_{min}$  where E is the exposure in ergs/cm<sup>2</sup>.

"Desktop Print Stability" is the formation of additional image or "print-out" when the imaged and processed film is stored for a period of time under given conditions of temperature, relative humidity, and light exposure. It is

usually most evident as an increase in  $D_{min}$ . Desktop Print Stability tends to be especially problematic under high humidity conditions. It is one type of post-processing stability.

"Aspect ratio" refers to the ratio of particle or grain "ECD" to particle or grain thickness wherein ECD (equivalent circular diameter) refers to the diameter of a circle having the same projected area as the particle or grain.

The phrase "organic silver coordinating ligand" refers to an organic molecule capable of forming a bond with a silver atom. Although the compounds so formed are technically silver coordination complexes or silver compounds they are also often referred to as silver salts.

In the compounds described herein, no particular double bond geometry (for example, cis or trans) is intended by the structures drawn unless otherwise specified. Similarly, in compounds having alternating single and double bonds and localized charges, their structures are drawn as a formalism. In reality, both electron and charge delocalization exist throughout the conjugated chain.

As is well understood in this art, for the chemical compounds herein described, substitution is not only tolerated, but is often advisable and various substituents are anticipated on the compounds used in the present invention unless otherwise stated. Thus, when a compound is referred to as "having the structure" of, or as "a derivative" of, a given formula, any substitution that does not alter the bond structure of the formula or the shown atoms within that structure is included within the formula, unless such substitution is specifically excluded by language.

As a means of simplifying the discussion and recitation of certain substituent groups, the term "group" refers to chemical species that may be substituted as well as those that are not so substituted. Thus, the term "alkyl group" is intended to include not only pure hydrocarbon alkyl chains, such as methyl, ethyl, n-propyl, t-butyl, cyclohexyl, iso-octyl, and octadecyl, but also alkyl chains bearing substituents known in the art, such as hydroxy, alkoxy, phenyl, halogen atoms (F, Cl, Br, and I), cyano, nitro, amino, and carboxy. For example, alkyl group includes ether and thioether groups (for example  $\text{CH}_3-\text{CH}_2-\text{CH}_2-\text{O}-\text{CH}_2-$  and  $\text{CH}_3-\text{CH}_2-\text{CH}_2-\text{S}-\text{CH}_2-$ ), hydroxyalkyl (such as 1,2-dihydroxyethyl), haloalkyl, nitroalkyl, alkylcarboxy, carboxyalkyl, carboxamido, sulfoalkyl, and other groups readily apparent to one skilled in the art. Substituents that adversely react with other active ingredients, such as very strongly electrophilic or oxidizing substituents, would, of course, be excluded by the ordinarily skilled artisan as not being inert or harmless.

*Research Disclosure* (<http://www.researchdisclosure.com>) is a publication of Kenneth Mason Publications Ltd., The Book Barn, Westbourne, Hampshire PO10 8RS, UK. It is also available from Emsworth Design Inc., 200 Park Avenue South, Room 1101, New York, N.Y. 10003.

Other aspects, advantages, and benefits of the present invention are apparent from the detailed description, examples, and claims provided in this application.

#### The Photocatalyst

The photothermographic materials include one or more photocatalysts in the photothermographic emulsion layer(s). Useful photocatalysts are typically photosensitive silver halides such as silver bromide, silver iodide, silver chloride, silver bromoiodide, silver chlorobromoiodide, silver chlorobromide, and others readily apparent to one skilled in the art. Mixtures of silver halides can also be used in any suitable proportion. Silver bromide and silver bromoiodide

are more preferred silver halides, with the latter silver halide having up to 100 mol % silver iodide (more preferably up to 40 mol %) silver iodide based on total silver halide, and up to the saturation limit of iodide as described in U.S. Patent Application Publication 2004/0053173 (Maskasky et al.).

The shape (morphology) of the photosensitive silver halide grains used in the present need not be limited. The silver halide grains may have any crystalline habit including cubic, octahedral, tetrahedral, orthorhombic, rhombic, dodecahedral, other polyhedral, tabular, laminar, twinned, or platelet morphologies and may have epitaxial growth of crystals thereon. If desired, a mixture of these crystals can be employed. Silver halide grains having cubic and tabular morphology (or both) are preferred. More preferably, the silver halide grains are predominantly (at least 50% based on total silver halide) present as tabular grains.

The silver halide grains may have a uniform ratio of halide throughout. They may have a graded halide content, with a continuously varying ratio of, for example, silver bromide and silver iodide or they may be of the core-shell type, having a discrete core of one or more silver halides, and a discrete shell of one of more different silver halides. Core-shell silver halide grains useful in photothermographic materials and methods of preparing these materials are described for example in U.S. Pat. No. 5,382,504 (Shor et al.), incorporated herein by reference. Iridium and/or copper doped core-shell and non-core-shell grains are described in U.S. Pat. No. 5,434,043 (Zou et al.) and U.S. Pat. No. 5,939,249 (Zou), both incorporated herein by reference.

In some instances, it may be helpful to prepare the photosensitive silver halide grains in the presence of a hydroxytetraazaindene or an N-heterocyclic compound comprising at least one mercapto group as described in U.S. Pat. No. 6,413,710 (Shor et al.), that is incorporated herein by reference.

The photosensitive silver halide can be added to (or formed within) the emulsion layer(s) in any fashion as long as it is placed in catalytic proximity to the non-photosensitive source of reducible silver ions.

It is preferred that the silver halide grains be preformed and prepared by an ex-situ process, chemically and spectrally sensitized, and then be added to and physically mixed with the non-photosensitive source of reducible silver ions.

It is also possible to form the source of reducible silver ions in the presence of ex-situ-prepared silver halide grains. In this process, the source of reducible silver ions is formed in the presence of the preformed silver halide grains. Precipitation of the reducible source of silver ions in the presence of silver halide provides a more intimate mixture of the two materials [see, for example U.S. Pat. No. 3,839,049 (Simons)] to provide a "preformed emulsion." This method is useful when non-tabular silver halide grains are used.

In general, the non-tabular silver halide grains used in this invention can vary in average diameter of up to several micrometers ( $\mu\text{m}$ ) and they usually have an average particle size of from about 0.01 to about 1.5  $\mu\text{m}$  (preferably from about 0.03 to about 1.0  $\mu\text{m}$ , and more preferably from about 0.05 to about 0.8  $\mu\text{m}$ ). The average size of the photosensitive silver halide grains is expressed by the average diameter if the grains are spherical, and by the average of the diameters of equivalent circles for the projected images if the grains are cubic, tabular, or other non-spherical shapes. Representative grain sizing methods are described by in *Particle Size Analysis*, ASTM Symposium on Light Microscopy, R. P. Loveland, 1955, pp. 94-122, and in C. E. K. Mees and T. H. James, *The Theory of the Photographic Process*, Third Edition, Macmillan, New York, 1966, Chapter 2.

In preferred embodiments of this invention, the silver halide grains are provided predominantly (based on at least 50 mol % silver) as tabular silver halide grains that are considered "ultrathin" and have an average thickness of at least 0.02  $\mu\text{m}$  and up to and including 0.10  $\mu\text{m}$  (preferably an average thickness of at least 0.03  $\mu\text{m}$  and more preferably of at least 0.04  $\mu\text{m}$ , and up to and including 0.08  $\mu\text{m}$  and more preferably up to and including 0.07  $\mu\text{m}$ ).

In addition, these ultrathin tabular grains have an equivalent circular diameter (ECD) of at least 0.5  $\mu\text{m}$  (preferably at least 0.75  $\mu\text{m}$ , and more preferably at least 1  $\mu\text{m}$ ). The ECD can be up to and including 8  $\mu\text{m}$  (preferably up to and including 6  $\mu\text{m}$ , and more preferably up to and including 4  $\mu\text{m}$ ).

The aspect ratio of the useful tabular grains is at least 5:1 (preferably at least 10:1, and more preferably at least 15:1) and generally up to 50:1. The grain size of ultrathin tabular grains may be determined by any of the methods commonly employed in the art for particle size measurement, such as those described above. Ultrathin tabular grains and their method of preparation and use in photothermographic materials are described in U.S. Pat. No. 6,576,410 (Zou et al.) and U.S. Pat. No. 6,673,529 (Dabendiek et al.) that are incorporated herein by reference.

The ultrathin tabular silver halide grains can also be doped using one or more of the conventional metal dopants known for this purpose including those described in *Research Disclosure* item 38957, September, 1996 and U.S. Pat. No. 5,503,970 (Olm et al.), incorporated herein by reference. Preferred dopants include iridium (III or IV) and ruthenium (II or III) salts. Particularly preferred silver halide grains are ultrathin tabular grains containing iridium-doped azole ligands. Such tabular grains and their method of preparation are described in copending and commonly assigned U.S. Ser. No. 10/826,708 (filed on Apr. 16, 2004 by Olm, McDugle, Hansen, Pawlik, Lewis, Mydlarz, Wilson, and Bell) that is incorporated herein by reference.

It is also possible to form some in-situ silver halide, by a process in which an inorganic halide- or an organic halogen-containing compound is added to an organic silver salt to partially convert the silver of the organic silver salt to silver halide as described in U.S. Pat. No. 3,457,075 (Morgan et al.).

The one or more light-sensitive silver halides used in the photothermographic materials are preferably present in an amount of from about 0.005 to about 0.5 mole (more preferably from about 0.01 to about 0.25 mole, and most preferably from about 0.03 to about 0.15 mole) per mole of non-photosensitive source of reducible silver ions.

#### Chemical Sensitizers

If desired, the photosensitive silver halides used in the photothermographic materials can be chemically sensitized using any useful compound that contains sulfur, tellurium, or selenium, or may comprise a compound containing gold, platinum, palladium, ruthenium, rhodium, iridium, or combinations thereof, a reducing agent such as a tin halide or a combination of any of these. The details of these materials are provided for example, in T. H. James, *The Theory of the Photographic Process*, Fourth Edition, Eastman Kodak Company, Rochester, N.Y., 1977, Chapter 5, pp. 149-169. Suitable conventional chemical sensitization procedures and compounds are also described in U.S. Pat. No. 1,623,499 (Sheppard et al.), U.S. Pat. No. 2,399,083 (Waller et al.), U.S. Pat. No. 3,297,447 (McVeigh), U.S. Pat. No. 3,297,446 (Dunn), U.S. Pat. No. 5,049,485 (Deaton), U.S. Pat. No. 5,252,455 (Deaton), U.S. Pat. No. 5,391,727 (Deaton), U.S.

## 11

Pat. No. 5,912,111 (Lok et al.), U.S. Pat. No. 5,759,761 (Lushington et al.), U.S. Pat. No. 6,296,998 (Eikenberry et al.), and U.S. Pat. No. 5,691,127 (Daubendiek et al.), and EP 0 915 371 A1 (Lok et al.), all incorporated herein by reference.

Certain substituted or and unsubstituted thioureas can be used as chemical sensitizers including those described in U.S. Pat. No. 6,296,998 (Eikenberry et al.), U.S. Pat. No. 6,322,961 (Lam et al.), U.S. Pat. No. 4,810,626 (Burgmaier et al.), and U.S. Pat. No. 6,368,779 (Lynch et al.), all of the which are incorporated herein by reference.

Still other useful chemical sensitizers include tellurium- and selenium-containing compounds that are described in U.S. Pat. No. 5,158,892 (Sasaki et al.), U.S. Pat. No. 5,238,807 (Sasaki et al.), U.S. Pat. No. 5,942,384 (Arai et al.) U.S. Pat. No. 6,620,577 (Lynch et al.), and U.S. Pat. No. 6,699,647 (Lynch et al.), all of which are incorporated herein by reference.

Noble metal sensitizers for use in the present invention include gold, platinum, palladium and iridium. Gold (I or III) sensitization is particularly preferred, and described in U.S. Pat. No. 5,858,637 (Eshelman et al.) and U.S. Pat. No. 5,759,761 (Lushington et al.). Combinations of gold (III) compounds and either sulfur- or tellurium-containing compounds are useful as chemical sensitizers and are described in U.S. Pat. No. 6,423,481 (Simpson et al.). All of the above references are incorporated herein by reference.

In addition, sulfur-containing compounds can be decomposed on silver halide grains in an oxidizing environment according to the teaching in U.S. Pat. No. 5,891,615 (Winslow et al.). Examples of sulfur-containing compounds that can be used in this fashion include sulfur-containing spectral sensitizing dyes.

Other useful sulfur-containing chemical sensitizing compounds that can be decomposed in an oxidized environment are the diphenylphosphine sulfide compounds described in copending and commonly assigned U.S. Ser. No. 10/731,251 (filed Dec. 9, 2003 by Simpson, Burleva, and Sakizadeh), incorporated herein by reference.

The chemical sensitizers can be used in making the silver halide emulsions in conventional amounts that generally depend upon the average size of silver halide grains. Generally, the total amount is at least  $10^{-10}$  mole per mole of total silver, and preferably from about  $10^{-8}$  to about  $10^{-2}$  mole per mole of total silver. The upper limit can vary depending upon the compound(s) used, the level of silver halide, and the average grain size and grain morphology.

#### Spectral Sensitizers

The photosensitive silver halides used in the photothermographic materials may be spectrally sensitized with one or more spectral sensitizing dyes that are known to enhance silver halide sensitivity to ultraviolet, visible, and/or infrared radiation of interest. Non-limiting examples of sensitizing dyes that can be employed include cyanine dyes, merocyanine dyes, complex cyanine dyes, complex merocyanine dyes, holopolar cyanine dyes, hemicyanine dyes, styryl dyes, and hemioxanol dyes. They may be added at any stage in chemical finishing of the photothermographic emulsion, but are generally added after chemical sensitization. It is particularly useful that the photosensitive silver halides be spectrally sensitized to a wavelength of from about 300 to about 850 nm, preferably from about 300 to about 600 nm, more preferably to a wavelength of from about 300 to about 450 nm, even more preferably from a wavelength of from about 360 to 420 nm, and most preferably from a wavelength of from about 380 to about 420 nm. In other embodi-

## 12

ments, the photosensitive silver halides are spectrally sensitized to a wavelength of from about 650 to about 1150 nm. A worker skilled in the art would know which dyes would provide the desired spectral sensitivity.

5 Suitable sensitizing dyes such as those described in U.S. Pat. No. 3,719,495 (Lea), U.S. Pat. No. 4,396,712 (Kinoshita et al.), U.S. Pat. No. 4,439,520 (Kofron et al.), U.S. Pat. No. 4,690,883 (Kubodera et al.), U.S. Pat. No. 4,840,882 (Iwagaki et al.), U.S. Pat. No. 5,064,753 (Kohno et al.), U.S. Pat. No. 5,281,515 (Delprato et al.), U.S. Pat. No. 5,393,654 (Burrows et al.), U.S. Pat. No. 5,441,866 (Miller et al.), U.S. Pat. No. 5,508,162 (Dankosh), U.S. Pat. No. 5,510,236 (Dankosh), and U.S. Pat. No. 5,541,054 (Miller et al.), and Japanese Kokai 2000-063690 (Tanaka et al.), 10 2000-112054 (Fukusaka et al.), 2000-273329 (Tanaka et al.), 2001-005145 (Arai), 2001-064527 (Oshiyama et al.), and 2001-154305 (Kita et al.), and *Research Disclosure*, item 15 308119, Section IV, December, 1989. All of these publications are incorporated herein by reference.

20 Teachings relating to specific combinations of spectral sensitizing dyes also provided in U.S. Pat. No. 4,581,329 (Sugimoto et al.), U.S. Pat. No. 4,582,786 (Ikeda et al.), U.S. Pat. No. 4,609,621 (Sugimoto et al.), U.S. Pat. No. 4,675,279 (Shuto et al.), U.S. Pat. No. 4,678,741 (Yamada et al.), U.S. Pat. No. 4,720,451 (Shuto et al.), U.S. Pat. No. 4,818,675 (Miayasa et al.), U.S. Pat. No. 4,945,036 (Arai et al.), and U.S. Pat. No. 4,952,491 (Nishikawa et al.), all of which are incorporated herein by reference.

25 Also useful are spectral sensitizing dyes that decolorize by the action of light or heat as described in U.S. Pat. No. 4,524,128 (Edwards et al.) and Japanese Kokai 2001-109101 (Adachi), 2001-154305 (Kita et al.), and 2001-183770 (Hanyu et al.), all of which are incorporated herein by reference.

30 Dyes may be selected for the purpose of supersensitization to attain much higher sensitivity than the sum of sensitivities that can be achieved by using each dye alone.

35 An appropriate amount of spectral sensitizing dye added 40 is generally about  $10^{-10}$  to  $10^{-1}$  mole, and preferably, from about  $10^{-7}$  to  $10^{-2}$  mole per mole of silver halide.

#### Non-Photosensitive Source of Reducible Silver Ions

45 The non-photosensitive source of reducible silver ions in the photothermographic materials is a silver-organic compound that contains reducible silver (I) ions. Such compounds are generally silver salts of silver organic coordinating ligands that are comparatively stable to light and form a silver image when heated to 50° C. or higher in the presence of an exposed photocatalyst and a reducing agent composition.

50 Organic silver salts that are particularly useful in photothermographic materials include silver salts of compounds containing an imino group. Such salts include, but are not 55 limited to, silver salts of benzotriazole and substituted derivatives thereof (for example, silver methylbenzotriazole and silver 5-chlorobenzotriazole), silver salts of nitrogen acids selected from the group consisting of imidazole, pyrazole, urazole, 1,2,4-triazole and 1H-tetrazole, nitrogen acids or combinations thereof, as described in U.S. Pat. No. 60 4,220,709 (deMauriac). Also included are the silver salts of imidazole and imidazole derivatives as described in U.S. Pat. No. 4,260,677 (Winslow et al.). Both of these patents are incorporated herein by reference. A nitrogen acid as 60 described herein is intended to include those compounds that have the moiety —NH— in the heterocyclic nucleus. Particularly useful silver salts are the silver salts of benzotriaz-

## 13

zole, substituted derivatives thereof, or mixtures of two or more of these salts. A silver salt of benzotriazole is most preferred.

Useful nitrogen-containing organic silver salts and methods of preparing them are also described in copending and commonly assigned U.S. Ser. No 10/826,417 (filed Apr. 16, 2004 by Zou and Hasberg) that is incorporated herein by reference. Such silver salts (particularly the silver benzotriazoles) are rod-like in shape and have an average aspect ratio of at least 3:1 and a width index for particle diameter of 1.25 or less. Silver salt particle length is generally less than 1  $\mu\text{m}$ . Also useful are silver salt-toner co-precipitated nano-crystals comprising a silver salt of a nitrogen-containing heterocyclic compound containing an imino group, and a silver salt comprising a silver salt of a mercaptotriazole as described in copending and commonly assigned U.S. Ser. No. 10/935,384 (filed Sep. 7, 2004 by Hasberg, Lynch, Chen-Ho, and Zou). Both of these patent applications are incorporated herein by reference.

Other organic silver salts that are useful in photothermographic materials are silver carboxylates (both aliphatic and aromatic carboxylates). The aliphatic carboxylic acids generally have aliphatic chains that contain 10 to 30. Silver salts of long-chain aliphatic carboxylic acids having 15 to 28 carbon atoms are particularly preferred. Examples of such preferred silver salts include silver behenate, silver arachidate, silver stearate, silver oleate, silver laurate, silver caprate, silver myristate, silver palmitate, silver maleate, silver fumarate, silver tartarate, silver furoate, silver linoleate, silver butyrate, silver camphorate, and mixtures thereof. Most preferably, at least silver behenate is used alone or in mixtures with other silver carboxylates. Silver carboxylates are particularly useful in organic solvent-based and aqueous latex-based photothermographic materials.

It is also convenient to use silver half soaps such as an equimolar blend of silver carboxylate and carboxylic acid that analyzes for about 14.5% by weight solids of silver in the blend and that is prepared by precipitation from an aqueous solution of an ammonium or an alkali metal salt of a commercially available fatty carboxylic acid, or by addition of the free fatty acid to the silver soap.

The methods used for making silver soap emulsions are well known in the art and are disclosed in *Research Disclosure*, April 1983, item 22812, *Research Disclosure*, October 1983, item 23419, U.S. Pat. No. 3,985,565 (Gabrielsen et al.) and the references cited above.

While the noted organic silver salts are the predominant silver salts in the materials, secondary organic silver salts can be used if present in "minor" amounts (less than 40 mol % based on the total moles of organic silver salts).

Such secondary organic silver salts include silver salts of heterocyclic compounds containing mercapto or thione groups and derivatives thereof such as silver triazoles, oxazoles, thiazoles, thiazolines, imidazoles, diazoles, pyridines, and triazines as described in U.S. Pat. No. 4,123,274 (Knight et al.) and U.S. Pat. No. 3,785,830 (Sullivan et al.). Also included are silver salts of aliphatic carboxylic acids containing a thioether group as described in U.S. Pat. No. 3,330,663 (Weyde et al.), soluble silver carboxylates comprising hydrocarbon chains incorporating ether or thioether linkages or sterically hindered substitution in the  $\alpha$ - (on a hydrocarbon group) or ortho- (on an aromatic group) position as described in U.S. Pat. No. 5,491,059 (Whitcomb), silver salts of dicarboxylic acids, silver salts of sulfonates as described in U.S. Pat. No. 4,504,575 (Lee), silver salts of sulfosuccinates as described in EP 0 227 141A1 (Leenders et al.), silver salts of aromatic carboxylic

## 14

acids (such as silver benzoate), silver salts of acetylenes as described, for example in U.S. Pat. No. 4,761,361 (Ozaki et al.) and U.S. Pat. No. 4,775,613 (Hirai et al.). Examples of other useful silver salts of mercapto or thione substituted compounds that do not contain a heterocyclic nucleus include silver salts of thioglycolic acids, dithiocarboxylic acids, and thioamides.

Sources of non-photosensitive reducible silver ions can also be in the form of core-shell silver salts as described in U.S. Pat. No. 6,355,408 (Whitcomb et al.) or the silver dimer compounds that comprise two different silver salts as described in U.S. Pat. No. 6,472,131 (Whitcomb), both references being incorporated herein by reference.

Still other useful sources of non-photosensitive reducible silver ions are the silver core-shell compounds comprising a primary core comprising one or more photosensitive silver halides, or one or more non-photosensitive inorganic metal salts or non-silver containing organic salts, and a shell at least partially covering the primary core, wherein the shell comprises one or more non-photosensitive silver salts, each of which silver salts comprises a organic silver coordinating ligand. Such compounds are described in U.S. Pat. No. 6,802,177 (Bokhonov et al.) that is incorporated herein by reference.

The one or more non-photosensitive sources of reducible silver ions (both primary and secondary organic silver salts) are preferably present in a total amount of about 5% by weight to about 70% by weight, and more preferably, about 10% to about 50% by weight, based on the total dry weight of the emulsion layers. Alternatively, the total amount of reducible silver ions is generally present in an amount of from about 0.001 to about 0.2 mol/m<sup>2</sup> of the dry photothermographic material (preferably from about 0.01 to about 0.05 mol/m<sup>2</sup>).

The total amount of silver (from all silver sources) in the photothermographic materials is generally at least 0.002 mol/m<sup>2</sup> and preferably from about 0.01 to about 0.05 mol/m<sup>2</sup> for single-sided materials. For double-sided coated materials, total amount of silver from all sources would be doubled.

## Reducing Agents

The reducing agent (or reducing agent composition comprising two or more components) for the source of reducible silver ions can be any material (preferably an organic material) that can reduce silver (I) ion to metallic silver. The "reducing agent" is sometimes called a "developer" or "developing agent."

When a silver benzotriazole silver source is used, ascorbic acid and reductone reducing agents are preferred. An "ascorbic acid" reducing agent means ascorbic acid, complexes, and derivatives thereof. Ascorbic acid reducing agents are described in a considerable number of publications including U.S. Pat. No. 5,236,816 (Purol et al.) and references cited therein.

Useful ascorbic acid developing agents include ascorbic acid and the analogues, isomers and derivatives thereof. Such compounds include, but are not limited to, D- or L-ascorbic acid, sugar-type derivatives thereof (such as sorboascorbic acid,  $\gamma$ -lactoascorbic acid, 6-desoxy-L-ascorbic acid, L-rhamno-ascorbic acid, imino-6-desoxy-L-ascorbic acid, glucoascorbic acid, fucoascorbic acid, glucohepatoascorbic acid, maltoascorbic acid, L-arabosascorbic acid), sodium ascorbate, potassium ascorbate, isoascorbic acid (or L-erythroascorbic acid), and salts thereof (such as alkali metal, ammonium or others known in the art), endiol type ascorbic acid, an enaminol type ascorbic acid, a thienoel

type ascorbic acid, and an enamine-thiol type ascorbic acid, as described in EP 0 585 792A1 (Passarella et al.), EP 0 573 700A1 (Lingier et al.), EP 0 588 408A1 (Hieronymus et al.), U.S. Pat. No. 5,089,819 (Knapp), U.S. Pat. No. 2,688,549 (James et al.), U.S. Pat. No. 5,278,035 (Knapp), U.S. Pat. No. 5,384,232 (Bishop et al.), U.S. Pat. No. 5,376,510 (Parker et al.), and U.S. Pat. No. 5,498,511 (Yamashita et al.), Japanese Kokai 7-56286 (Toyoda), and *Research Disclosure*, item 37152, March 1995. Mixtures of these developing agents can be used if desired.

Particularly useful reducing agents are ascorbic acid mono- or di-fatty acid esters such as the monolaurate, monomyristate, monopalmitate, monostearate, monobehenate, diluarate, distearate, dipalmitate, dibehenate, and dimyristate derivatives of ascorbic acid as described in U.S. Pat. No. 3,832,186 (Masuda et al.) and U.S. Pat. No. 6,309,814 (Ito). Preferred ascorbic acid reducing agents and their methods of preparation are those described in copending and commonly assigned U.S. Ser. No. 10/764,704 (filed on Jan. 26, 2004 by Ramsden, Lynch, Skoug, and Philip) and U.S. Ser. No. 10/935,645 (filed on Sep. 7, 2004 by Brick, Ramsden, and Lynch), both of which are incorporated herein by reference. A preferred reducing agent is L-ascorbic acid 6-O-palmitate.

A "reductone" reducing agent means a class of unsaturated, di- or poly-enolic organic compounds that, by virtue of the arrangement of the enolic hydroxy groups with respect to the unsaturated linkages, possess characteristic strong reducing power. The parent compound, "reductone" is 3-hydroxy-2-oxo-propionaldehyde (enol form) and has the structure HOCH=CH(OH)—CHO. Examples of reductone reducing agents can be found in U.S. Pat. No. 2,691,589 (Henn et al.), U.S. Pat. No. 3,615,440 (Bloom), U.S. Pat. No. 3,664,835 (Youngquist et al.), U.S. Pat. No. 3,672,896 (Gabrielson et al.), U.S. Pat. No. 3,690,872 (Gabrielson et al.), U.S. Pat. No. 3,816,137 (Gabrielson et al.), U.S. Pat. No. 4,371,603 (Bartels-Keith et al.), U.S. Pat. No. 5,712,081 (Andriesen et al.), and U.S. Pat. No. 5,427,905 (Freedman et al.), all of which references are incorporated herein by reference.

When a silver carboxylate silver source is used in a photothermographic material, one or more hindered phenol reducing agents are preferred. In some instances, the reducing agent composition comprises two or more components such as a hindered phenol developer and a co-developer that can be chosen from the various classes of co-developers and reducing agents described below. Ternary developer mixtures involving the further addition of contrast enhancing agents are also useful. Such contrast enhancing agents can be chosen from the various classes of reducing agents described below.

"Hindered phenol reducing agents" are compounds that contain only one hydroxy group on a given phenyl ring and have at least one additional substituent located ortho to the hydroxy group.

One type of hindered phenol reducing agent includes hindered phenols and hindered naphthols.

Another type of hindered phenol reducing agent are hindered bis-phenols. These compounds contain more than one hydroxy group each of which is located on a different phenyl ring. This type of hindered phenol includes, for example, binaphthols (that is dihydroxybinaphthyls), biphenols (that is dihydroxybiphenyls), bis(hydroxynaphthyl) methanes, bis(hydroxyphenyl)-methanes bis(hydroxyphenyl)ethers, bis(hydroxyphenyl)sulfones, and bis(hydroxyphenyl)thioethers, each of which may have additional substituents.

Preferred hindered phenol reducing agents are bis(hydroxyphenyl)methanes such as, bis(2-hydroxy-3-t-butyl-5-methylphenyl)methane (CAO-5), 1,1'-bis(2-hydroxy-3,5-dimethylphenyl)-3,5,5-trimethylhexane (NONOX® or PERMANAX WSO), and 1,1'-bis(2-hydroxy-3,5-dimethylphenyl)-isobutane (LOWINOX® 22IB46). Mixtures of hindered phenol reducing agents can be used if desired.

An additional class of reducing agents that can be used includes substituted hydrazines including the sulfonyl hydrazides described in U.S. Pat. No. 5,464,738 (Lynch et al.). Still other useful reducing agents are described in U.S. Pat. No. 3,074,809 (Owen), U.S. Pat. No. 3,094,417 (Workman), U.S. Pat. No. 3,080,254 (Grant, Jr.), U.S. Pat. No. 3,887,417 (Klein et al.), and U.S. Pat. No. 5,981,151 (Leenders et al.). All of these patents are incorporated herein by reference.

Additional reducing agents that may be used include amidoximes, azines, a combination of aliphatic carboxylic acid aryl hydrazides and ascorbic acid, a reductone and/or a hydrazine, piperidinohexose reductone or formyl-4-methylphenylhydrazine, hydroxamic acids, a combination of azines and sulfonamidophenols,  $\alpha$ -cyanophenylacetic acid derivatives, reductones, indane-1,3-diones, chromans, 1,4-dihydropyridines, and 3-pyrazolidones.

Useful co-developer reducing agents can also be used as described in U.S. Pat. No. 6,387,605 (Lynch et al.) U.S. Pat. No. 5,496,695 (Simpson et al.), U.S. Pat. No. 5,654,130 (Murray), U.S. Pat. No. 5,705,324 (Murray), U.S. Pat. No. 6,100,022 (Inoue et al.), U.S. Pat. No. 5,635,339 (Murray), and U.S. Pat. No. 5,545,515 (Murray et al.). All of the patents above are incorporated herein by reference.

Various contrast enhancing agents can be used in some photothermographic materials with specific co-developers. Examples of useful contrast enhancing agents include, but are not limited to, hydroxamic acid compounds, N-acylhydrazine compounds, hydrogen donor compounds, hydroxylamines, alkanolamines and ammonium phthalamate compounds as described in U.S. Pat. No. 5,545,505 (Simpson), U.S. Pat. No. 5,545,507 (Simpson et al.), U.S. Pat. No. 5,558,983 (Simpson et al.), and U.S. Pat. No. 5,637,449 (Harring et al.), all of which are incorporated herein by reference.

The reducing agent (or mixture thereof) described herein is generally present as 1 to 10% (dry weight) of the emulsion layer. In multilayer constructions, if the reducing agent is added to a layer other than an emulsion layer, slightly higher proportions, of from about 2 to 15 weight % may be more desirable. Co-developers may be present generally in an amount of from about 0.001% to about 1.5% (dry weight) of the emulsion layer coating.

#### Blocked Aliphatic Thiol Compounds

The blocked aliphatic thiol compounds useful in the invention have a "c log P" value high enough to improve Desktop Print Stability in a photothermographic formulation compared to the formulation without the compound. Preferably the c log P value is 2 or greater. More preferably, the c log P value is 5 or greater.

The c log P value is a calculated estimate of the octanol-water partition coefficient (P), which is a physical property used extensively to describe a chemical's lipophilic or hydrophobic properties. It is the ratio of a chemical's concentration in the octanol-phase to its concentration in the aqueous-phase of a two-phase system at equilibrium. Since measured values range from  $<10^{-4}$  to  $>10^{+8}$  (at least 12 orders of magnitude), the logarithm (log P) is commonly used to characterize its value. The Log Octanol-Water Par-

tion Coefficient Program KOWWIN<sup>®</sup> may be used to estimate the logarithmic octanol-water partition coefficient (log P) of organic compounds. This program is available from the U.S. Environmental Protection Agency via free internet download from the web-page <www.epa.gov/oppt/exposure/docs/episuitedl.htm>. KOWWIN<sup>®</sup> requires only a chemical structure to estimate log P values. Structures are entered into KOWWIN<sup>®</sup> by SMILES (Simplified Molecular Input Line Entry System) notations. The KOWWIN<sup>®</sup> program and estimation methodology were developed by W. Meylan of Syracuse Research Corporation (North Syracuse, N.Y.), and is described in W. M. Meylan and P. H. Howard, *J. Pharm. Sci.* 1995, 84, 83-92 entitled *Atom/fragment Method for Estimating Octanol-Water Partition Coefficients*. All values for "c log P" used herein were calculated using KOWWIN<sup>®</sup> Version 1.661.

The blocked aliphatic thiol compounds useful in the invention also have an "N Value" equal to or greater than 6.5, and preferably greater than 12. The N Value is the total number of atoms in the "thiol portion" of the blocked aliphatic thiol compound minus the number of hydrogen atoms in the "thiol portion", that is, the number of "non-hydrogen atoms in the "thiol portion," divided by the number of blocked aliphatic thiol groups. An equation for this ratio is given below. By "thiol portion", we mean the aliphatic thiol that is released by the thermal de-blocking of the blocked aliphatic thiol. In the case of an aliphatic polythiol, the "thiol portion" would refer to complete de-blocking of all of the blocking groups.

$$N \text{ Value} = \frac{\text{Number of Non-Hydrogen Atoms in the Released Thiol}}{\text{Number of Blocked Aliphatic Thiol Groups}}$$

In preferred embodiments, the blocked aliphatic thiol compounds can be represented by the following Structures (I) or (II):



wherein R<sub>1</sub> is a substituted or unsubstituted mono- or multivalent aliphatic group, BLOCK-1 is a monovalent thermally releasing blocking group, BLOCK-2 is a multivalent thermally releasing blocking group, m is an integer from 2 to 4, and n is an integer from 1 to 4. Preferred examples of monovalent thermally releasing blocking groups (BLOCK-1) include the following Structures (III), (IV), (V), and (VI). Preferred examples of a multivalent thermally releasing blocking group (BLOCK-2) include the following Structures (VII) and (VIII):



-continued



wherein R<sub>2</sub> is hydrogen, a substituted or unsubstituted aliphatic, heterocyclic, or (hetero)aromatic group, a R<sub>3</sub>SO<sub>2</sub>— group, or a R<sub>3</sub>—(C=O)— group, wherein R<sub>3</sub> is a substituted or unsubstituted aliphatic, heterocyclic, or (hetero) aromatic group, R<sub>4</sub>, R<sub>5</sub>, and R<sub>6</sub> are the same or different and are hydrogen or a substituted or unsubstituted aliphatic, heterocyclic, or (hetero)aromatic group, R<sub>7</sub> is a substituted or unsubstituted tertiary alkyl or tertiary aralkyl group, X<sub>2</sub> is R<sub>2</sub>—, HO—, H<sub>2</sub>N—, R<sub>2</sub>O—, R<sub>2</sub>S—, R<sub>2</sub>NH—, or R<sub>2</sub>R<sub>3</sub>N—, X<sub>1</sub> is oxygen or sulfur, R<sub>8</sub> is a multivalent substituted or unsubstituted aliphatic, heterocyclic, or (hetero)aromatic group, Y<sup>—</sup> is an anion sufficient to neutralize the positive charge, and \* designates the point of attachment of the thermally releasing blocking group to the sulfur of the thiol, with the proviso that any of R<sub>2</sub>, R<sub>3</sub>, R<sub>4</sub>, R<sub>5</sub>, R<sub>6</sub>, and X<sub>2</sub> may be linked to one another to form a (polycyclic)ring.

Preferred examples of R<sub>2</sub> groups include substituted and unsubstituted phenyl and naphthyl groups, substituted and unsubstituted alkyl groups having 4 to 18 carbon atoms, and substituted or unsubstituted alkyl- and aryl-sulfonyl groups. More preferred examples of R<sub>2</sub> groups include phenyl, 4-chlorophenyl, 3-chlorophenyl, 4-cyanophenyl, 2-naphthyl, butyl, hexyl, cyclohexyl, and 4-tolyl sulfonyl.

Preferred examples of R<sub>3</sub> groups include substituted and unsubstituted phenyl and naphthyl groups, and substituted and unsubstituted alkyl groups having 4 to 18 carbon atoms. More preferred examples of R<sub>3</sub> groups include, phenyl, 4-chlorophenyl, 3-chlorophenyl, 4-cyanophenyl, 2-naphthyl, butyl, and hexyl.

Preferred examples of R<sub>4</sub>, R<sub>5</sub>, and R<sub>6</sub> groups include hydrogen, substituted and unsubstituted phenyl and naphthyl groups, and substituted and unsubstituted alkyl groups having 4 to 18 carbon atoms. More preferred examples of R<sub>4</sub>, R<sub>5</sub>, and R<sub>6</sub> groups include hydrogen, phenyl, 4-chlorophenyl, 3-chlorophenyl, 4-cyanophenyl, 2-naphthyl, butyl, and hexyl.

Preferred examples of R<sub>7</sub> groups include tertiary alkyl groups having from 4 to 8 carbon atoms and tertiary benzyl groups having from 9 to 12 carbon atoms. More preferred examples of R<sub>7</sub> groups include tertiary-butyl, tertiary-pentyl, and α,α-dimethylbenzyl.

Preferred examples of R<sub>8</sub> groups include substituted and unsubstituted phenylene groups, substituted or unsubstituted alkylidene groups having 4 to 18 carbon atoms, and methyldiynetri-p-phenylene groups. More preferred examples of

19

R<sub>8</sub> groups include 1,4-phenylene, 2,4-tolylene-, 4,4'-methylenebisphenyl, 1,6-hexylidene, dicyclohexylmethane 4,4'-diyl, and methylidynetri-p-phenylene groups.

A preferred example of X<sub>1</sub> is oxygen. Preferred examples of X<sub>2</sub> groups include substituted and unsubstituted alkyl groups having 1 to 4 carbon atoms, substituted and unsubstituted phenyl groups, HO—, and R<sub>2</sub>O—. More preferred examples of X<sub>2</sub> groups are hydrogen, phenyl, 4-chlorophenyl, 3-chlorophenyl, methoxy, and ethoxy. 5

Preferred examples of Y<sup>-</sup> groups include tetrafluoroborate, halide, tosylate, and hexafluorophosphate. A more preferred example is tetrafluoroborate. 10

Preferred examples of R<sub>1</sub> groups include substituted or unsubstituted alkyl groups having 10 to 24 carbon atoms, 15 R<sub>9</sub>O<sub>2</sub>CCH<sub>2</sub>—, R<sub>9</sub>O<sub>2</sub>CCH<sub>2</sub>CH<sub>2</sub>—, R<sub>9</sub>NHCONHCH<sub>2</sub>CH<sub>2</sub>—, R<sub>9</sub>CONHCH<sub>2</sub>CH<sub>2</sub>—, R<sub>9</sub>SO<sub>2</sub>NHCH<sub>2</sub>CH<sub>2</sub>—, alkyl benzyl groups, 20 R<sub>9</sub>NHCO<sub>2</sub>CH<sub>2</sub>CH<sub>2</sub>, and R<sub>9</sub>O<sub>2</sub>CNHCH<sub>2</sub>CH<sub>2</sub>R<sub>9</sub> is an alkyl or aryl group having 6 or more carbon atoms. Preferred examples of R<sub>9</sub> include pentadecyl, hexadecyl, heptadecyl, and octadecyl. More preferred examples of R<sub>1</sub> groups include substituted or unsubstituted hexadecyl, heptadecyl, octadecyl, eicosanyl, uncosyl, docosyl, 12-phenyldodecyl, 25 10-hexyloxydecyl, 18-methoxyoctadecyl, 16-methylthiohexadecyl, 18-methyloctadecyl, 4-octylbenzyl, and 3,3,4,4, 5,5,6,6,7,7,8,8,9,9,10,10,10-heptadecylfluorodecyl, C<sub>16</sub>H<sub>32</sub>O<sub>2</sub>CCH<sub>2</sub>CH<sub>2</sub>—, and C<sub>16</sub>H<sub>32</sub>CONHCH<sub>2</sub>CH<sub>2</sub>— groups. 30

Preferred values of n are 1 and 2 (more preferably, n is 1). Preferred values of m are 2 and 3 (more preferably, m is 2).

Representative blocked aliphatic thiol compounds useful in the practice of the present invention include the following compounds PS-1 through PS-47: 35

20

-continued

(PS-6)



(PS-7)



(PS-8)



(PS-9)



(PS-10)



(PS-11)



(PS-12)



(PS-13)



(PS-14)



(PS-15)



(PS-1)

40

(PS-2)

45

(PS-3)

50

(PS-4)

55

(PS-5)

60

(PS-6)

(PS-7)

65

(PS-8)

(PS-9)

**21**

-continued



(PS-16)



(PS-17)



(PS-18)



(PS-19)



(PS-20)



(PS-21)



(PS-22)



(PS-23)



(PS-24)

**22**

-continued

(PS-25)



(PS-26)



(PS-27)



(PS-28)



(PS-29)



(PS-30)



(PS-31)



(PS-32)



(PS-33)



(PS-34)



(PS-35)



-continued



-continued

(PS-36) (PS-47)



Upon development, compounds (I) and (II) decompose by cleavage of the S-BLOCK bond to release aliphatic thiol compounds  $R_1-SH$  or  $R_1-(SH)_n$  that act as Desktop Print Stabilizers for photothermographic materials.

In general, the blocked aliphatic thiol compounds useful in this invention represented by Structures (I) and (II) can be prepared by known methods, such as the reaction of a thiol with an isocyanate, the reaction of a thiol with phosgene, the reaction of a thiol with an  $\alpha,\beta$ -unsaturated carbonyl compound, the reaction of a thiol with an isothiocyanate, the reaction of a thiol with thiophosgene, and other reactions readily apparent to one skilled in the art. Representative preparations of several PS-Compounds are given in the Examples Section below.

The preferred blocked aliphatic thiol compounds include PS-1, PS-2, PS-3, PS-8, and PS-34, and Compound PS-3 is most preferred.

The noted blocked aliphatic thiol compounds can be present in the photothermographic material in an amount of at least 1 mg/m<sup>2</sup> and preferably from about 5 mg/m<sup>2</sup> to about 500 mg/m<sup>2</sup>, and more preferably from about 5 mg/m<sup>2</sup> to about 100 mg/m<sup>2</sup>. Two or more of these compounds can be used if desired.

Other Addenda

The photothermographic materials can also contain other additives such as toners, additional shelf-life stabilizers, antifogging agents, contrast enhancing agents, development accelerators, acutance dyes, additional post-processing stabilizers or stabilizer precursors, thermal solvents (also known as melt formers), humectants, and other image-modifying agents as would be readily apparent to one skilled in the art.

Toners are compounds that shift the color of the developed silver image from yellowish-orange to brown-black or blue-black, and/or act as development accelerators to speed up thermal development. "Toners" or derivatives thereof that improve the black-and-white image are highly desirable components of the photothermographic materials.

Thus, compounds that either act as toners or react with a reducing agent to provide toners can be present in an amount of about 0.01% by weight to about 10% (preferably from about 0.1% to about 10% by weight) based on the total dry weight of the layer in which they are included. The amount can also be defined as being within the range of from about  $1 \times 10^{-5}$  to about 1.0 mol per mole of non-photosensitive source of reducible silver in the photothermographic material. The toner compounds may be incorporated in one or more of the photothermographic layers as well as in adjacent layers such as the outermost protective layer or underlying "carrier" layer. Toners can be located on both sides of the support if photothermographic layers are present on both sides of the support.

Compounds useful as toners are described in U.S. Pat. No. 3,074,809 (Owen), U.S. Pat. No. 3,080,254 (Grant, Jr.), U.S. Pat. No. 3,446,648 (Workman), U.S. Pat. No. 3,844,797 (Willems et al.), U.S. Pat. No. 3,847,612 (Winslow), U.S.

Pat. No. 3,951,660 (Hagemann et al.), U.S. Pat. No. 4,082,901 (Laridon et al.), U.S. Pat. No. 4,123,282 (Winslow), U.S. Pat. No. 5,599,647 (Defieuw et al.), and U.S. Pat. No. 3,832,186 (Masuda et al.), and GB 1,439,478 (AGFA).

Particularly useful toners are mercaptotriazoles as described in U.S. Pat. No. 6,713,240 (Lynch et al.), the heterocyclic disulfide compounds described in U.S. Pat. No. 6,737,227 (Lynch et al.), the triazine-thione compounds described in U.S. Pat. No. 6,703,191 (Lynch et al.), and the silver salt-toner co-precipitated nano-crystals described in copending and commonly assigned U.S. Ser. No. 10/935,384 (noted above). All of the above are incorporated herein by reference.

Also useful as toners are phthalazine and phthalazine derivatives [such as those described in U.S. Pat. No. 6,146,822 (Asanuma et al.) incorporated herein by reference], phthalazinone, and phthalazinone derivatives as well as phthalazinium compounds [such as those described in U.S. Pat. No. 6,605,418 (Ramsden et al.), incorporated herein by reference].

To further control the properties of photothermographic materials, (for example, contrast,  $D_{min}$ , speed, or fog), it may be preferable to add one or more heteroaromatic mercapto compounds or heteroaromatic disulfide compounds of the formulae  $\text{Ar}-\text{S}-\text{M}^1$  and  $\text{Ar}-\text{S}-\text{S}-\text{Ar}$ , wherein  $\text{M}^1$  represents a hydrogen atom or an alkali metal atom and  $\text{Ar}$  represents a heteroaromatic ring or fused heteroaromatic ring containing one or more of nitrogen, sulfur, oxygen, selenium, or tellurium atoms. Useful heteroaromatic mercapto compounds are described as supersensitizers in EP 0 559 228 B1 (Philip Jr. et al.).

The photothermographic materials can be further protected against the production of fog and can be stabilized against loss of sensitivity during storage. Suitable antifoggants and stabilizers that can be used alone or in combination include thiazolium salts as described in U.S. Pat. No. 2,131,038 (Brooker et al.) and U.S. Pat. No. 2,694,716 (Allen), azaindenes as described in U.S. Pat. No. 2,886,437 (Piper), triazaindolizines as described in U.S. Pat. No. 2,444,605 (Heimbach), urazoles as described in U.S. Pat. No. 3,287,135 (Anderson), sulfocatechols as described in U.S. Pat. No. 3,235,652 (Kennard), oximes as described in GB 623,448 (Carroll et al.), polyvalent metal salts as described in U.S. Pat. No. 2,839,405 (Jones), and the thiuronium salts as described in U.S. Pat. No. 3,220,839 (Herz).

The photothermographic materials may also include one or more polyhalo antifoggants that include one or more polyhalo substituents including but not limited to, dichloro, dibromo, trichloro, and tribromo groups. The antifoggants can be aliphatic, alicyclic or aromatic compounds, including aromatic heterocyclic and carbocyclic compounds. Particularly useful antifoggants of this type are polyhalo antifoggants, such as those having a  $-\text{SO}_2\text{C}(\text{X}')_3$  group wherein  $\text{X}'$  represents the same or different halogen atoms. Such compounds are described, for example, in U.S. Pat. No. 5,460,938 (Kirk et al.), U.S. Pat. No. 5,594,143 (Kirk et al.), and U.S. Pat. No. 5,374,514 (Kirk et al.).

Another class of useful antifoggants includes those compounds described in U.S. Pat. No. 6,514,678 (Burgmaier et al.), incorporated herein by reference.

Advantageously, the photothermographic materials also include one or more thermal solvents (also called "heat solvents," "thermosolvents," "melt formers," "melt modifiers," "eutectic formers," "development modifiers," "waxes," or "plasticizers"). By the term "thermal solvent" is meant an organic material that becomes a plasticizer or liquid solvent

for at least one of the imaging layers upon heating at a temperature above 60° C. Representative examples of such compounds include polyethylene glycols having a mean molecular weight in the range of 1,500 to 20,000, ethylene carbonate, niacinamide, hydantoin, 5,5-dimethylhydantoin, salicylanilide, succinimide, phthalimide, N-potassium-phthalimide, N-hydroxyphthalimide, N-hydroxy-1,8-naphthalimide, phthalazine, 1-(2H)-phthalazinone, 2-acetylphthalazinone, benzanilide, urea, 1,3-dimethylurea, 1,3-diethylurea, 1,3-diallylurea, meso-erythritol, D-sorbitol, tetrahydro-2-pyrimidone, glycouril, 2-imidazolidone, 2-imidazolidone-4-carboxylic acid, methyl sulfonamide, and benzenesulfonamide. Combinations of these compounds can also be used including, for example, a combination of succinimide and 1,3-dimethylurea. Known thermal solvents are disclosed, for example, in U.S. Pat. No. 3,347,675 (Henn et al.), U.S. Pat. No. 3,438,776 (Yudelson), U.S. Pat. No. 5,250,386 (Aono et al.), U.S. Pat. No. 5,368,979 (Freedman et al.), U.S. Pat. No. 5,716,772 (Taguchi et al.), and U.S. Pat. No. 6,013,420 (Windender), and in *Research Disclosure*, December 1976, item 15027. All of these are incorporated herein by reference.

It may also be advantageous to include one or more "boron" compounds in the photothermographic materials with the blocked aliphatic thiol compounds. "Boron" compounds can be represented by the following Structure (IX):



wherein X and Z are independently hydroxy, alkoxy, alkyl, acyl, or aryl groups, L is hydrogen, alkyl, aryl, or heteroaryl, or X and Z together represent carbon or heteroatoms sufficient to provide a heterocyclic ring with the boron atom, or still again, X, L, and Z together represent carbon or heteroatoms sufficient to provide a heterocyclic ring with the boron atom.

Preferred boron compounds include boric acid and boric acid esters (such as, trimethylborate, triisopropylborate, tris(2,4-dimethyl-3-pentyl)-borate, and the borate ester of triisopropanolamine). More details are provided in copending and commonly assigned U.S. Ser. No. 11/025,882 (filed on even date herewith by Philip, Lynch, Ramsden, Klaus, and Ulrich) entitled "Boron Compounds As Stabilizers In Photothermographic Materials," and incorporated herein by reference.

#### Phosphors

In some embodiments, it is also effective to incorporate X-radiation-sensitive phosphors in the photothermographic materials as described in U.S. Pat. No. 6,573,033 (Simpson et al.) and U.S. Pat. No. 6,440,649 (Simpson et al.), both of which are incorporated herein by reference. Other useful phosphors are primarily "activated" phosphors known as phosphate phosphors and borate phosphors. Examples of these phosphors are rare earth phosphates, yttrium phosphates, strontium phosphates, or strontium fluoroborates (including cerium activated rare earth or yttrium phosphates, or europium activated strontium fluoroborates) as described in U.S. Ser. No. 10/826,500 (filed Apr. 16, 2004 by Simpson, Sieber, and Hansen).

The one or more phosphors used in the practice of this invention are present in the photothermographic materials in an amount of at least 0.1 mole per mole of total silver in the photothermographic material.

#### Binders

The photosensitive silver halide, the non-photosensitive source of reducible silver ions, the reducing agent, antifog-

gant(s), and any other additives used in the present invention are added to and coated in one or more binders using a suitable aqueous or non-aqueous solvent. Thus, aqueous-based formulations can be used to prepare the photothermographic materials. Mixtures of different types of hydrophilic and/or hydrophobic binders can also be used. Preferably, hydrophilic polymer binders and water-dispersible polymeric latexes are used to provide aqueous-based formulations and photothermographic materials. Alternatively, hydrophobic binders can be used to provide non-aqueous based formulations and photothermographic materials.

Examples of useful hydrophilic polymer binders include, but are not limited to, proteins and protein derivatives, gelatin and gelatin derivatives (hardened or unhardened), cellulosic materials, acrylamide/methacrylamide polymers, acrylic/methacrylic polymers, polyvinyl pyrrolidones, polyvinyl alcohols, poly(vinyl lactams), polymers of sulfoalkyl acrylate or methacrylates, hydrolyzed polyvinyl acetates, polyamides, polysaccharides, and other naturally occurring or synthetic vehicles commonly known for use in aqueous-based photographic emulsions (see for example *Research Disclosure*, item 38957, noted above). Minor amounts (less than 50 weight % based on total binder weight) of hydrophobic binders (not in latex form) may also be used.

Particularly useful hydrophilic polymer binders are gelatin, gelatin derivatives, polyvinyl alcohols, and cellulosic materials. Gelatin and its derivatives are most preferred, and comprise at least 75 weight % of total binders when a mixture of binders is used.

Aqueous dispersions of water-dispersible polymeric latexes may also be used, alone or with hydrophilic or hydrophobic binders described herein. Such dispersions are described in, for example, U.S. Pat. No. 4,504,575 (Lee), U.S. Pat. No. 6,083,680 (Ito et al.), U.S. Pat. No. 6,100,022 (Inoue et al.), U.S. Pat. No. 6,132,949 (Fujita et al.), U.S. Pat. No. 6,132,950 (Ishigaki et al.), U.S. Pat. No. 6,140,038 (Ishizuka et al.), U.S. Pat. No. 6,150,084 (Ito et al.), U.S. Pat. No. 6,312,885 (Fujita et al.), and U.S. Pat. No. 6,423,487 (Naoh), all of which are incorporated herein by reference.

Examples of typical hydrophobic binders include polyvinyl acetals, polyvinyl chloride, polyvinyl acetate, cellulose acetate, cellulose acetate butyrate, polyolefins, polyesters, polystyrenes, polyacrylonitrile, polycarbonates, methacrylate copolymers, maleic anhydride ester copolymers, butadiene-styrene copolymers, and other materials readily apparent to one skilled in the art. The polyvinyl acetals (such as polyvinyl butyral and polyvinyl formal), cellulose ester polymers, and vinyl copolymers (such as polyvinyl acetate and polyvinyl chloride) are preferred. Particularly suitable binders are polyvinyl butyral resins that are available under the name BUTVAR® from Solutia, Inc. (St. Louis, Mo.) and PIOLOFORM® from Wacker Chemical Company (Adrian, Mich.) and cellulose ester polymers.

Hardeners for various binders may be present if desired. Useful hardeners are well known and include diisocyanates as described for example, in EP 0 600 586B1 (Philip, Jr. et al.) and vinyl sulfone compounds as described in U.S. Pat. No. 6,143,487 (Philip, Jr. et al.), and EP 0 640 589A1 (Gathmann et al.), aldehydes and various other hardeners as described in U.S. Pat. No. 6,190,822 (Dickerson et al.).

Where the proportions and activities of the photothermographic materials require a particular developing time and temperature, the binder(s) should be able to withstand those conditions. Generally, it is preferred that the binder does not decompose or lose its structural integrity at 120° C. for 60

seconds. It is more preferred that it does not decompose or lose its structural integrity at 177° C. for 60 seconds.

The binder(s) is used in an amount sufficient to carry the components dispersed therein. Preferably, a binder is used at a level of about 10% by weight to about 90% by weight, and more preferably at a level of about 20% by weight to about 70% by weight, based on the total dry weight of the layer in which it is included. The amount of binders on opposing sides of the support in double-sided materials may be the same or different.

#### Support Materials

The photothermographic materials comprise a polymeric support that is preferably a flexible, transparent film that has any desired thickness and is composed of one or more polymeric materials. They are required to exhibit dimensional stability during thermal development and to have suitable adhesive properties with overlying layers. Useful polymeric materials for making such supports include, but are not limited to, polyesters, cellulose acetate and other cellulose esters, polyvinyl acetal, polyolefins, polycarbonates, and polystyrenes. Preferred supports are composed of polymers having good heat stability, such as polyesters and polycarbonates. Polyethylene terephthalate film is a particularly preferred support. Support materials may also be treated or annealed to reduce shrinkage and promote dimensional stability.

It is also useful to use supports comprising dichroic mirror layers as described in U.S. Pat. No. 5,795,708 (Boutet), incorporated herein by reference.

Also useful are transparent, multilayer, polymeric supports comprising numerous alternating layers of at least two different polymeric materials as described in U.S. Pat. No. 6,630,283 (Simpson et al.) that is incorporated herein by reference.

Support materials can contain various colorants, pigments, antihalation or acutance dyes if desired. For example, blue-tinted supports are particularly useful for providing images useful for medical diagnosis. Support materials may be treated using conventional procedures (such as corona discharge) to improve adhesion of overlying layers, or subbing or other adhesion-promoting layers can be used.

#### Photothermographic Formulations and Constructions

The imaging components are prepared in a formulation containing a polymer binder (such as gelatin, a gelatin-derivative, a cellulosic material, or a polyvinyl butyral) or a water-dispersible polymer in latex form in an aqueous or non-aqueous solvent (or mixtures thereof) to provide coating formulations. The photothermographic imaging layers on one or both sides of the support are coated out of these formulations.

The photothermographic materials can contain plasticizers and lubricants such as poly(alcohols) and diols as described in U.S. Pat. No. 2,960,404 (Milton et al.), fatty acids or esters as described in U.S. Pat. No. 2,588,765 (Robijns) and U.S. Pat. No. 3,121,060 (Duane), and silicone resins as described in GB 955,061 (DuPont). The materials can also contain inorganic or organic matting agents as described in U.S. Pat. No. 2,992,101 (Jolley et al.) and U.S. Pat. No. 2,701,245 (Lynn). Polymeric fluorinated surfactants may also be useful in one or more layers as described in U.S. Pat. No. 5,468,603 (Kub).

U.S. Pat. No. 6,436,616 (Geisler et al.), incorporated herein by reference, describes various means of modifying photothermographic materials to reduce what is known as the "woodgrain" effect, or uneven optical density.

The photothermographic materials can include one or more antistatic agents in any of the layers on either or both sides of the support. Conductive components include soluble salts, evaporated metal layers, or ionic polymers as described in U.S. Pat. No. 2,861,056 (Minsk) and U.S. Pat. No. 3,206,312 (Sterman et al.), insoluble inorganic salts as described in U.S. Pat. No. 3,428,451 (Trevoy), poly-thiophenes as described in U.S. Pat. No. 5,747,412 (Leenders et al.), electro-conductive underlayers as described in U.S. Pat. No. 5,310,640 (Markin et al.), electronically-conductive metal antimonate particles as described in U.S. Pat. No. 5,368,995 (Christian et al.), and electrically-conductive metal-containing particles dispersed in a polymeric binder as described in EP 0 678 776 A1 (Melpolder et al.). Particularly useful conductive particles are the non-acicular metal antimonate particles described in U.S. Pat. No. 6,689,546 (LaBelle et al.), and in copending and commonly assigned U.S. Ser. No. 10/930,428 (filed Aug. 31, 2004 by Ludemann, LaBelle, Koestner, Hefley, Bhave, Geisler, and Philip), Ser. No. 10/930,438 (filed Aug. 31, 2004 by Ludemann, LaBelle, Philip, Koestner, and Bhave), and Ser. No. 10/978,205 (filed Oct. 29, 2004 by Ludemann, LaBelle, Koestner, and Chen). All of the above patents and patent applications are incorporated herein by reference.

In addition, fluorochemicals such as Fluorad® FC-135 (3M Corporation), ZONYL® FSN (E. I. DuPont de Nemours & Co.), as well as those described in U.S. Pat. No. 5,674,671 (Brandon et al.), U.S. Pat. No. 6,287,754 (Melpolder et al.), U.S. Pat. No. 4,975,363 (Cavallo et al.), U.S. Pat. No. 6,171,707 (Gomez et al.), and U.S. Pat. No. 6,699,648 (Sakizadeh et al.), and U.S. Pat. No. 6,762,013 (Sakizadeh et al.) can be used. All of the above are incorporated herein by reference.

The photothermographic materials can have a protective overcoat layer (or outermost overcoat layer) disposed over the one or more imaging layers on one or both sides of the support. The binders for such overcoat layers can be any of the binders described in the Binders Section. Preferably, the protective layers include gelatin or a gelatin derivative as the predominant binder(s) especially when the one or more imaging layers also include gelatin or a gelatin derivative as the predominant binder(s). Alternatively, the protective layers include a cellulosic ester (such as cellulose acetate butyrate) when the predominant binder is polyvinylbutyral.

For double-sided photothermographic materials, each side of the support can include one or more of the same or different imaging layers, interlayers, and protective overcoat layers. In such materials preferably a overcoat is present as the outermost layer on both sides of the support. The photothermographic layers on opposite sides can have the same or different construction and can be overcoated with the same or different protective layers.

Layers to promote adhesion of one layer to another are also known, as described in U.S. Pat. No. 5,891,610 (Bauer et al.), U.S. Pat. No. 5,804,365 (Bauer et al.), and U.S. Pat. No. 4,741,992 (Przezdziecki). Adhesion can also be promoted using specific polymeric adhesive materials as described for example in U.S. Pat. No. 5,928,857 (Geisler et al.).

Layers to reduce emissions from the film may also be present, including the polymeric barrier layers described in U.S. Pat. No. 6,352,819 (Kenney et al.), U.S. Pat. No. 6,352,820 (Bauer et al.), U.S. Pat. No. 6,420,102 (Bauer et al.), U.S. Pat. No. 6,667,148 (Rao et al.), and U.S. Pat. No. 6,746,831 (Hunt), all incorporated herein by reference.

The formulations described herein (including the photothermographic formulations) can be coated by various coat-

ing procedures including wire wound rod coating, dip coating, air knife coating, curtain coating, slide coating, or extrusion coating using hoppers of the type described in U.S. Pat. No. 2,681,294 (Beguin). Layers can be coated one at a time, or two or more layers can be coated simultaneously by the procedures described in U.S. Pat. No. 2,761,791 (Russell), U.S. Pat. No. 4,001,024 (Dittman et al.), U.S. Pat. No. 4,569,863 (Keopke et al.), U.S. Pat. No. 5,340,613 (Hanzalik et al.), U.S. Pat. No. 5,405,740 (LaBelle), U.S. Pat. No. 5,415,993 (Hanzalik et al.), U.S. Pat. No. 5,525,376 (Leonard), U.S. Pat. No. 5,733,608 (Kessel et al.), U.S. Pat. No. 5,849,363 (Yapel et al.), U.S. Pat. No. 5,843,530 (Jerry et al.), and U.S. Pat. 5,861,195 (Bhave et al.), and GB 837,095 (Ilford). A typical coating gap for the emulsion layer can be from about 10 to about 750  $\mu$ m, and the layer can be dried in forced air at a temperature of from about 20° C. to about 100° C. It is preferred that the thickness of the layer be selected to provide maximum image densities greater than about 0.2, and more preferably, from about 0.5 to 5.0 or more, as measured by a MacBeth Color Densitometer Model TD 504.

Simultaneously with or subsequently to application of an emulsion formulation to the support, a protective overcoat formulation can be applied over the emulsion formulation.

Preferably, two or more layer formulations are applied simultaneously to a film support using slide coating techniques, the overcoat layer being coated on top of the photothermographic emulsion layer while the photothermographic emulsion layer is still wet.

In other embodiments, a "carrier" layer formulation comprising a single-phase mixture of the two or more polymers may be applied directly onto the support and thereby located underneath the emulsion layer(s) as described in U.S. Pat. No. 6,355,405 (Ludemann et al.), incorporated herein by reference. The carrier layer formulation can be applied simultaneously with application of the photothermographic emulsion layer formulation and any overcoat formulations.

Mottle and other surface anomalies can be reduced in the materials by incorporation of a fluorinated polymer as described in U.S. Pat. No. 5,532,121 (Yonkoski et al.) or by using particular drying techniques as described in U.S. Pat. No. 5,621,983 (Ludemann et al.).

While the overcoat and photothermographic layers can be coated on one side of the film support, manufacturing methods can also include forming on the opposing or backside of the polymeric support, one or more additional layers, including a conductive layer, antihalation layer, or a layer containing a matting agent (such as silica), or a combination of such layers. Alternatively, one backside layer can perform all of the desired functions.

To promote image sharpness, photothermographic materials can contain one or more layers containing acutance and/or antihalation dyes that are chosen to have absorption close to the exposure wavelength and are designed to absorb scattered light. One or more antihalation compositions may be incorporated into one or more antihalation backing layers, antihalation underlayers, or as antihalation overcoats.

Dyes useful as antihalation and acutance dyes include squaraine dyes described in U.S. Pat. No. 5,380,635 (Gomez et al.) and U.S. Pat. No. 6,063,560 (Suzuki et al.), and EP 1 083 459A1 (Kimura), indolenine dyes described in EP 0 342 810A1 (Leichter), and cyanine dyes described in U.S. Pat. No. 6,689,547 (Hunt et al.), all incorporated herein by reference.

It may also be useful to employ compositions including acutance or antihalation dyes that will decolorize or bleach with heat during processing, as described in U.S. Pat. No.

5,135,842 (Kitchin et al.), U.S. Pat. No. 5,266,452 (Kitchin et al.), U.S. Pat. No. 5,314,795 (Helland et al.), and U.S. Pat. No. 6,306,566, (Sakurada et al.), and Japanese Kokai 2001-142175 (Hanyu et al.) and 2001-183770 (Hanyu et al.). Useful bleaching compositions are also described in Japanese Kokai 11-302550 (Fujiwara), 2001-109101 (Adachi), 2001-51371 (Yabuki et al.), and 2000-029168 (Noro). All of the noted publications are incorporated herein by reference.

Other useful heat-bleachable backside antihalation compositions can include an infrared radiation absorbing compound such as an oxonol dye or other compounds used in combination with a hexaarylbiiimidazole (also known as a "HABI"), or mixtures thereof. HABI compounds are described in U.S. Pat. No. 4,196,002 (Levinson et al.), U.S. Pat. No. 5,652,091 (Perry et al.), and U.S. Pat. No. 5,672,562 (Perry et al.), all incorporated herein by reference. Examples of such heat-bleachable compositions are described for example in U.S. Pat. No. 6,455,210 (Irving et al.), U.S. Pat. No. 6,514,677 (Ramsden et al.), and U.S. Pat. No. 6,558,880 (Goswami et al.), all incorporated herein by reference.

Under practical conditions of use, these compositions are heated to provide bleaching at a temperature of at least 90° C. for at least 0.5 seconds (preferably, at a temperature of from about 100° C. to about 200° C. for from about 5 to about 20 seconds).

#### Imaging/Development

The photothermographic materials can be imaged in any suitable manner consistent with the type of material, using any suitable imaging source (typically some type of radiation or electronic signal). In some embodiments, the materials are sensitive to radiation in the range of from about at least 100 nm to about 1400 nm, and normally from about 300 nm to about 750 nm (preferably from about 300 to about 600 nm, more preferably from about 300 to about 450 nm, even more preferably from a wavelength of from about 360 to 420 nm, and most preferably from about 380 to about 420 nm), using appropriate spectral sensitizing dyes.

Imaging can be achieved by exposing the photothermographic materials to a suitable source of radiation to which they are sensitive, including ultraviolet radiation, visible light, near infrared radiation, and infrared radiation to provide a latent image. Suitable exposure means are well known and include incandescent or fluorescent lamps, xenon flash lamps, lasers, laser diodes, light emitting diodes, infrared lasers, infrared laser diodes, infrared light-emitting diodes, infrared lamps, or any other ultraviolet, visible, or infrared radiation source readily apparent to one skilled in the art such as described in *Research Disclosure*, item 38957 (noted above).

In preferred embodiments, the photothermographic materials can be indirectly imaged using an X-radiation imaging source and one or more prompt-emitting or storage X-ray sensitive phosphor screens adjacent to the photothermographic material. The phosphors emit suitable radiation to expose the photothermographic material. Preferred X-ray screens are those having phosphors emitting in the near ultraviolet region of the spectrum (from 300 to 400 nm), in the blue region of the spectrum (from 400 to 500 nm) and those emitting in the green region of the spectrum (from 500 to 600 nm).

In other embodiments, the photothermographic materials can be imaged directly using an X-radiation imaging source to provide a latent image.

Thermal development conditions will vary, depending on the construction used but will typically involve heating the photothermographic material at a suitably elevated tempera-

ture, for example, at from about 50° C. to about 250° C. (preferably from about 80° C. to about 200° C. and more preferably from about 100° C. to about 200° C.) for a sufficient period of time, generally from about 1 to about 120 seconds. Heating can be accomplished using any suitable heating means. A preferred heat development procedure for photothermographic materials includes heating at from 130° C. to about 165° C. for from about 3 to about 25 seconds.

#### 10 Use as a Photomask

In some embodiments, the photothermographic materials are sufficiently transmissive in the range of from about 350 to about 450 nm in non-imaged areas to allow their use in a method where there is a subsequent exposure of an ultraviolet or short wavelength visible radiation sensitive imageable medium. The heat-developed materials absorb ultraviolet or short wavelength visible radiation in the areas where there is a visible image and transmit ultraviolet or short wavelength visible radiation where there is no visible image. 15 The materials may then be used as a mask and positioned between a source of imaging radiation (such as an ultraviolet or short wavelength visible radiation energy source) and an imageable material that is sensitive to such imaging radiation, such as a photopolymer, diazo material, photoresist, or 20 photosensitive printing plate.

These embodiments of the imaging method of this invention are carried out using steps (A) and (B) noted above with the following Steps (C) and (D):

- 30 (C) positioning the exposed and photothermographic material with the visible image therein between a source of imaging radiation and an imageable material that is sensitive to the imaging radiation, and  
 35 (D) exposing the imageable material to the imaging radiation through the visible image in the exposed and photothermographic material to provide an image in the imageable material.

#### Imaging Assemblies

40 In some embodiments, the photothermographic materials are used or arranged in association with one or more phosphor intensifying screens and/or metal screens in what is known as "imaging assemblies." Duplitized visible light sensitive photothermographic materials are preferably used in combination with two adjacent intensifying screens, one screen in the "front" and one screen in the "back" of the material. The front and back screens can be appropriately chosen depending upon the type of emissions desired, the desired photicity, and emulsion speeds. The imaging assemblies can be prepared by arranging the photothermographic material and one or more phosphor intensifying screens in a suitable holder (often known as a cassette), and appropriately packaging them for transport and imaging uses.

45 There are a wide variety of phosphors known in the art that can be formulated into phosphor intensifying screens as described in hundreds of publications. U.S. Pat. No. 6,573, 033 (noted above) describes phosphors that can be used in this manner. Particularly useful phosphors are those that emit radiation having a wavelength of from about 300 to about 450 nm and preferably radiation having a wavelength of from about 360 to about 420 nm.

50 Preferred phosphors useful in the phosphor intensifying screens include one or more alkaline earth fluorohalide phosphors and especially the rare earth activated (doped) alkaline earth fluorohalide phosphors. Particularly useful phosphor intensifying screens include a europium-doped barium fluorobromide (BaFBr<sub>2</sub>:Eu) phosphor. Other useful

33

phosphors are described in U.S. Pat. No. 6,682,868 (Dickerson et al.) and references cited therein, all incorporated herein by reference.

The following examples are provided to illustrate the practice of the present invention and the invention is not meant to be limited thereby.

#### Materials and Methods for the Examples:

All materials used in the following examples can be prepared using known synthetic procedures or are available from standard commercial sources, such as Aldrich Chemical Co. (Milwaukee, Wis.), unless otherwise specified. All percentages are by weight unless otherwise indicated. The following additional materials were prepared and used.

BYK-022 is a defoamer and is available from Byk-Chemie Corp. (Wallingford, Conn.).

BZT is benzotriazole. AGBZT is silver benzotriazole. NaBZT is the sodium salt of benzotriazole.

CELVOL® 203S is a poly(vinyl alcohol) (PVA) and is available from Celanese Corp. (Dallas, Tex.).

SPP 3000 is an 88% hydrolyzed poly(vinyl alcohol) having a molecular weight of 3000. It is available from Scientific Polymer Products. (Ontario, N.Y.).

TRITON® X-114 is a nonionic surfactant that is available from Dow Chemical Corp. (Midland Mich.).

TRITON® X-200 is an anionic surfactant that is available from Dow Chemical Corp. (Midland Mich.).

ZONYL® FS-300 is a nonionic fluorosurfactant that is available from E. I. DuPont de Nemours & Co. (Wilmington, Del.).

Developer D-1 is L-Ascorbic acid 6-O-palmitate and is available from Aceto Corp., (Lake Success, N.Y.). It is believed to have the following structure.



Compound A-2 is described in U.S. Pat. No. 6,605,418 (Ramsden et al.) and is believed to have the following structure.



Compound SS-1a is described in U.S. Pat. No. 6,296,998 (Eikenberry et al.) and is believed to have the following structure:

5

34

(SS-1a)



Gold (III) chemical sensitizer Compound GS-1 is believed to have the following structure.

10

15

20

(GS-1)



Blue spectral sensitizing dye SSD-1 is believed to have the following structure.

30

35

40

(SSD-1)



45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

45

34

35

36

37

38

39

40

41

42

43

44

45

46

47

48

49

50

51

52

53

54

55

56

57

58

59

60

61

62

63

64

65

66

67

68

69

70

71

72

73

74

75

76

77

78

79

80

81

82

83

84

85

86

87

88

89

90

91

92

93

94

95

96

97

98

99

100

101

102

103

104

105

106

107

108

109

110

111

112

113

114

115

116

117

118

119

120

121

122

123

124

125

126

127

128

129

130

131

132

133

134

135

136

## Comparative Compounds:

Comparative compound C-1 has the structure shown below.



Comparative compound C-2 has the structure shown below. 15



Comparative compound C-3 has the structure shown below.



Comparative compound C4 has the structure shown below.



## Preparation of Blocked Aliphatic Thiols:

### Preparation of Compound PS-1:

To a mixture of 15.69 g (54.8 mmol) of octadecanethiol, 250 ml of acetonitrile, and 5 ml (4.9 g, 62 mmol) of pyridine and under a nitrogen atmosphere, 6.52 g (0.548 mmol) of phenylisocyanate were added all at once. The mixture was heated to reflux for 2 hours, then cooled to room temperature. The product crystallized, was collected by filtration, and was recrystallized from acetonitrile to give 19.19 g of S-octadecyl phenylcarbamothioate (Compound PS-1), mp 85.5–86.5° C.

Additional PS-Compounds were prepared in an analogous manner by reaction of the appropriate isocyanate with the appropriate aliphatic thiol. Their melting points are given below in TABLE I.

### Preparation of Compound PS-32:

1-Octadecanethiol (5.72 g, 0.02 mol) was dissolved in 50 ml of warm methanol. Phenylisothiocyanate (2.7 g, 0.02 mol) was added and the mixture was stirred overnight at

room temperature under a nitrogen atmosphere. Ethanol (100 ml) was added and the mixture heated till a clear yellow solution was obtained. Upon standing at room temperature,

crystals were formed. Yield 5.3 g (63%), mp 76–77° C. Thin layer chromatography (in ethyl acetate) showed one spot. Mass spectra gave the correct values, 422.3 in Positive mode and 420.2 in negative mode.

### Preparation of Compound PS-33:

Compound PS-33 was prepared by modification of the method described by Degani et al. (I. Degani, R. Fochi, and V. Regondi, *Synthesis*, 1980, (5), 375-378.).

A mixture of 1-bromoocadecane (33.3 g, 0.1 mol), potassium O-methyl dithiocarbonate<sup>a</sup> (17.0 g, 0.13 mol), tricaprylmethylammonium chloride (Aliquat 336®, Fluka, 3.4 g), and water (100 ml) was vigorously stirred at room temperature for 40 minutes<sup>b</sup>. The mixture was then extracted with diethyl ether, the extract was washed with water (2x30 ml), and the solvent evaporated in vacuo at 45° C. To the crude residue was added 100 ml of 2% sodium carbonate solution and the mixture was vigorously stirred at 50° C. for about 4 hours. The organic layer was extracted with diethyl ether and dried over sodium sulfate. Solvent was removed using a rotary evaporator at 70° C. The residue was dissolved in hot carbon tetrachloride and ethanol was added. Upon standing at room temperature crystals were formed. Yield 43 g (72%), mp 62–63°. <sup>1</sup>H— and <sup>13</sup>C-nmr spectra of the compound were consistent with that of desired product.

<sup>a</sup> Potassium O-methyl dithiocarbonate (potassium xanthate) was prepared by the reaction of potassium hydroxide, absolute ethanol, and carbon disulfide according to the general method described in *Vogel's Textbook of Practical Organic Chemistry*, Fifth Edition, Longman Scientific & Technical, Essex, England, 1989, p 793.

*b.* Gentle warming was required at the beginning of the reaction in order to dissolve the solid.

### Preparation of Compound PS-36:

To a solution of 10.40 g (50.0 mmol) of chalcone in 500 ml of methanol was added 1.8 ml of 1M tetrabutylammonium hydroxide in methanol. This was followed by portion-wise addition of 13.61 g (47.5 mmol) of octadecane thiol with good stirring. The product crystallized and was collected by filtration. Recrystallization from acetonitrile, followed by recrystallization from acetone gave 15.77 g of compound PS-36, mp 73–75° C.

TABLE I

| Compound | Melting Point (° C.) |
|----------|----------------------|
| PS-1     | 85.5–86.5            |
| PS-2     | 72–74                |
| PS-3     | 101–104              |
| PS-4     | 77–81                |
| PS-5     | 83–85                |
| PS-6     | 82–84.5              |
| PS-7     | 132–135              |
| PS-8     | 133–135              |
| PS-9     | 72–74                |
| PS-10    | 71–72                |

TABLE I-continued

| Compound | Melting Point (° C.) |
|----------|----------------------|
| PS-11    | 60-62                |
| PS-12    | 150-154              |
| PS-13    | 89-92                |
| PS-14    | 123-124.5            |
| PS-15    | 152-153.5            |
| PS-16    | 45-47                |
| PS-17    | 206                  |
| PS-18    | 90-91                |
| PS-19    | 76                   |
| PS-20    | 83-87                |
| PS-21    | 144-146              |
| PS-22    | 129                  |
| PS-23    | 113-114              |
| PS-24    | 109-111              |
| PS-25    | 119-120              |
| PS-26    | 90-92                |
| PS-27    | 92-94                |
| PS-28    | 103.5-105            |
| PS-29    | 94.5-96              |
| PS-30    | 126-129              |
| PS-31    | 91-92                |
| PS-32    | 76-77                |
| PS-33    | 62-63                |
| PS-34    | 148-149.5            |
| PS-35    | 95-97                |
| PS-36    | 73-75                |
| PS-37    | 99-100.5             |
| PS-38    | 102-105              |
| PS-40    | 72-73                |
| PS-41    | 61-63                |
| PS-42    | 65-67                |
| PS-43    | 78-79                |
| PS-44    | 74-77                |
| C-1      | 154-155              |
| C-2      | 74-77                |
| C-3      | 50-51                |

## EXAMPLE 1

## Preparation of Aqueous-Based Photothermographic Material:

An aqueous-based photothermographic material of this invention was prepared in the following manner.

## Preparation of Developer (D-1) Dispersions:

Aqueous slurries were prepared containing Developer D-1, CELVOL® 203S, poly(vinyl alcohol), TRITON® X-114 surfactant, and BYK-022. The poly(vinyl alcohol), TRITON®X-114 surfactant, and BYK-022 were added at a level of 10.0%, 3.0%, and 0.1% by weight to that of Developer D-1, respectively. The mixture was milled with 0.7 mm zirconium ceramic beads for about 7 hours. Examination of the final dispersion by transmitted light microscopy at 1000 $\times$  magnification showed well-dispersed particles, all below 1  $\mu$ m.

## Preparation of Blocked Aliphatic Thiol Dispersion:

A solid particle dispersion of blocked aliphatic thiol compound was prepared by combining 10 parts PS-Compound, 2.7 parts of SPP 3000 poly(vinyl alcohol), 0.05 parts of TRITON® X-200 surfactant, and 87.25 parts of deionized water. The mixture was milled using a micro media mill with 0.7 mm zirconium silicate ceramic beads for 90 minutes at 2000 rpm. This mill is described in U.S. Pat. No. 5,593,097 (Corbin) incorporated herein by reference. Filtration gave an aqueous dispersion containing 10% blocked thiol compound, with average particle size less than 1 micron.

## Preparation of AgBZT/AgT-1 Co-Precipitated Emulsion:

A co-precipitated AgBZT/AgT-1 emulsion was prepared as described in copending and commonly assigned U.S. Ser. No. 10/935,384 (noted above).

5 A stirred reaction vessel was charged with 900 g of lime-processed gelatin, and 6000 g of deionized water. The mixture in the reaction vessel was adjusted to a pH of 8.9 with 2.5N sodium hydroxide solution, and 0.8 g of Solution A (prepared below) was added to adjust the solution vAg to 10 80 mV. The temperature of the reaction vessel was maintained at approximately 50° C.

Solution A was prepared containing 216 g/kg of benzotriazole, 710 g/kg of deionized water, and 74 g/kg of sodium hydroxide.

15 Solution B was prepared containing 362 g/kg of silver nitrate and 638 g/kg of deionized water.

Solution C was prepared containing 336 g/kg of T-1, 70 g/kg of sodium hydroxide and 594 g/kg of deionized water.

Solutions A and B were then added to the reaction vessel 20 by conventional controlled double-jet addition. Solution B was continuously added at the flow rates and for the times given below, while maintaining constant vAg and pH in the reaction vessel. After consumption of 97.4% total silver nitrate solution (Solution B), Solution A was replaced with 25 Solution C and the precipitation was continued. Solution B and Solution C were added to the reaction vessel also by conventional controlled double-jet addition, while maintaining constant vAg and pH in the reaction vessel.

The AgBZT/AgT-1 co-precipitated emulsions were 30 washed by conventional ultrafiltration process as described in *Research Disclosure*, Vol. 131, March 1975, Item 13122. The pH of AgBZT/AgT-1 emulsions was adjusted to 6.0 using 2.0N sulfuric acid. Upon cooling the emulsion solidified and was stored.

35

|             | Time<br>[min] | Solution B Flow Rate<br>[ml/min] |
|-------------|---------------|----------------------------------|
| Flow Rate 1 | 20            | 25                               |
| Flow Rate 2 | 41            | 25-40                            |
| Flow Rate 3 | 30            | 40-80                            |

## Preparation of Ultra-Thin Tabular Grain Silver Halide Emulsion:

45 A reaction vessel equipped with a stirrer was charged with 6 liters of water containing 2.1 g of deionized oxidized-methionine lime-processed bone gelatin, 3.49 g of sodium bromide, and an antifoamant (at pH=5.8). The solution was held at 39° C. for 5 minutes. Simultaneous additions were 50 then made of 50.6 ml of 0.3 molar silver nitrate and 33.2 ml of 0.448 molar sodium bromide over 1 minute. Following nucleation, 3.0 ml of a 0.1 M solution of sulfuric acid was added. After 1 minute 15.62 g sodium chloride plus 375 mg 55 of sodium thiocyanate were added and the temperature was increased to 54° C. over 9 minutes. After a 5-minute hold, 79.6 g of deionized oxidized-methionine lime-processed bone gelatin in 1.52 liters of water containing additional antifoamant at 54° C. were then added to the reactor. The reactor temperature was held for 7 minutes (pH=5.6).

60 During the next 36.8 minutes, the first growth stage took place (at 54° C.), in three segments, wherein solutions of 0.3 molar AgNO<sub>3</sub>, 0.448 molar sodium bromide, and a 0.16 molar suspension of silver iodide (Lippmann) were added to maintain a nominal uniform iodide level of 3.2 mole %. The flow rates during this growth stage were increased from 9 to 42 ml/min (silver nitrate) and from 0.73 to 3.3 ml/min (silver

iodide). The flow rates of the sodium bromide were allowed to fluctuate as needed to affect a monotonic pBr shift of 2.45 to 2.12 over the first 12 minutes, of 2.12 to 1.90 over the second 12 minutes, and of 1.90 to 1.67 over the last 12.8 minutes. This was followed by a 1.5-minute hold.

During the next 59 minutes the second growth stage took place (at 54° C.) during which solutions of 2.8 molar silver nitrate, and 3.0 molar sodium bromide, and a 0.16 molar suspension of silver iodide (Lippmann) were added to maintain a nominal iodide level of 3.2 mole %. The flow rates during this segment were increased from 10 to 39.6 ml/min (silver nitrate) and from 5.3 to 22.6 ml/min (silver iodide). The flow rates of the sodium bromide were allowed to fluctuate as needed to affect a monotonic pBr shift of 1.67 to 1.50. This was followed by a 1.5-minute hold.

During the next 34.95 minutes, the third growth stage took place during which solutions of 2.8 molar silver nitrate, 3.0 molar sodium bromide, and a 0.16 molar suspension of silver iodide (Lippmann) were added to maintain a nominal iodide level of 3.2 mole %. The flow rates during this segment were 39.6 ml/min (silver nitrate) and 22.6 ml/min (silver iodide). The temperature was linearly decreased to 35° C. during this segment. At the 23<sup>rd</sup> minute of this segment a 50 ml aqueous solution containing 0.85 mg of an Iridium dopant ( $K_2[Ir(5-Br-thiazole)Cl_5]$ ) was added. The flow rate of the sodium bromide was allowed to fluctuate to maintain a constant pBr of 1.50.

A total of 8.5 moles of silver iodobromide (3.2% bulk iodide) were formed. The resulting emulsion was washed using ultrafiltration. Deionized lime-processed bone gelatin (326.9 g) was added along with a biocide and pH and pBr were adjusted to 6 and 2.5 respectively.

The resulting emulsion was examined by Scanning Electron Microscopy. Tabular grains accounted for greater than 99% of the total projected area. The mean ECD of the grains was 2.522  $\mu$ m. The mean tabular thickness was 0.049  $\mu$ m.

This emulsion was spectrally sensitized with 3.31 mmol of blue sensitizing dye SSD-1 per mole of silver halide. This dye quantity was split 80%/20% with the majority being added before chemical sensitization and the remainder afterwards. Chemical sensitization was carried out using 0.0085 mmol of sulfur sensitizer (compound SS-1a) and 0.00079 mmol per mole of silver halide of gold sensitizer (compound GS-1) at 60° C. for 6.3 minutes.

#### Preparation of Photothermographic Materials:

Component A: The AgBZT/AgT-1 co-precipitated emulsion prepared above and hydrated gelatin (35% gelatin/65% water) were placed in a beaker and heated to 50° C. for 15 minutes. A 5% aqueous solution of 3-methyl-benzothiazolium iodide was added and the mixture was heated for 15 minutes at 50° C. A 0.73 molar aqueous solution of sodium salt of benzotriazole was added and the mixture was heated for 10 minutes at 50° C. The mixture was cooled to 40° C. and its pH was adjusted to 5.0 with 2.5N sulfuric acid. A 18% aqueous solution of A-2 was added and the mixture was heated for 10 minutes at 40° C. A 4% active aqueous solution of ZONYL® FS-300 surfactant was then added and the mixture was held at 40° C.

Component B: A portion of the ultra-thin tabular grain silver halide emulsion prepared above was placed in a beaker and melted at 40° C.

Component C: A mixture of 1,3-dimethylurea, succinimide, and pentaerythritol was dissolved in water by heating at 50° C. The dispersion of D-1 described above was added to the above solution at room temperature.

Component D: A dispersion of the blocked thiol was prepared as described above.

Component E: A portion of hydrated gelatin (23% deionized lime-processed gelatin/77% water) was placed in a beaker and heated to 40° C. for 10 minutes to melt. The melt was added a 20% aqueous solution of 1,3-dimethylurea, a 5% aqueous solution of boric acid, and a 4% active aqueous solution of ZONYL® FS-300 surfactant.

Component F: A 1.7% aqueous solution of compound VS-1 was prepared by dissolving VS-1 in water at 50° C.

10 Coating and Evaluation of Photothermographic Materials: Components A, B, C, and D were mixed immediately before coating to form a photothermographic emulsion formulation, and components E and F were mixed immediately before coating to form a overcoat formulation. The photothermographic formulation and the overcoat formulation were coated as a dual layer on a 7 mil (178  $\mu$ m) transparent, blue-tinted poly(ethylene terephthalate) film support using a conventional automated dual-knife coating machine. The coating gaps for both layers were adjusted to achieve the dry coating weights shown in TABLE II. Samples were dried at 120° F. (48.9° C.) for 9 minutes. Inventive Samples 1-5-I through 1-27-I containing a dispersion of the indicated blocked thiol are shown in TABLE III. Comparative Samples 1-1-C through 1-4-C, were also prepared as shown in TABLE III.

TABLE II

| Component                | Compound                          | Dry Coating Weight (g/m <sup>2</sup> ) |
|--------------------------|-----------------------------------|----------------------------------------|
| Photothermographic Layer |                                   |                                        |
| 35 A                     | Silver (from AgBZT/AgT-1)         | 1.53                                   |
| A                        | Lime processed gelatin            | 2.34                                   |
| A                        | 3-Methylbenzothiazolium Iodide    | 0.077                                  |
| A                        | Sodium benzotriazole              | 0.092                                  |
| A                        | Compound A-2                      | 0.078                                  |
| A                        | ZONYL® FS-300 surfactant          | 0.022                                  |
| 40 B                     | Silver (from AgBrI emulsion)      | 0.27                                   |
| C                        | Succinimide                       | 0.19                                   |
| C                        | 1,3-Dimethylurea                  | 0.31                                   |
| C                        | Pentaerythritol                   | 0.50                                   |
| C                        | Developer D-1                     | 3.97                                   |
| D                        | Blocked Thiol Compound            | See TABLE III                          |
| Overcoat Layer           |                                   |                                        |
| 45 E                     | De-ionized lime-processed gelatin | 1.40                                   |
| E                        | Boric acid                        | 0.046                                  |
| E                        | 1,3-Dimethylurea                  | 0.19                                   |
| E                        | ZONYL® FS-300 surfactant          | 0.070                                  |
| F                        | Compound VS-1                     | 0.083                                  |

50 The resulting photothermographic films were imagewise exposed for  $10^{-2}$  seconds using an EG&G flash sensitometer equipped with a P-16 filter and a 0.7 neutral density filter. Following exposure, the films were developed on a heated flat bed for 18 seconds at 150° C. to generate continuous tone wedges. These samples provided initial  $D_{min}$ ,  $D_{max}$ , and Relative Speed-2 and are shown in TABLE III.

55 Densitometry measurements were made on a custom built computer-scanned densitometer meeting ISO Standards 5-2 and 5-3 and are believed to be comparable to measurements from commercially available densitometers. Density of the wedges was measured with the above-noted computer densitometer using a filter appropriate to the sensitivity of the photothermographic material to obtain graphs of density versus log exposure (that is, D log E curves).  $D_{min}$  is the

density of the non-exposed areas after development and it is the average of the eight lowest density values. Relative Speed-2 is determined at a density value of 1.00 above  $D_{min}$  and then normalized against sample 1-1-C, which contained no blocked aliphatic thiol compound and was assigned a relative speed value of 100.

Desktop Print Stability Test: Imaged and developed samples of each film were illuminated with 100 foot-candles (1076 lux) at 70° F. (21.2° C.) and 80% relative humidity (RH) for 24 hours. The  $D_{min}$  of each sample was measured both before and after illumination using an X-Rite® Model 301 densitometer (X-Rite Inc. Grandville, Mich.) equipped with a visible filter having a transmittance peak at about 530 nm. The change in visual density ( $\Delta D_{min}$ ) was calculated by subtracting the  $D_{min}$  of the initial sample from the  $D_{min}$  of sample after being subjected to light, heat, and humidity.

The results, shown below in TABLE III, demonstrate that the compounds of the present invention provide excellent Desktop Print Stability (that is, a lower  $\Delta D_{min}$ ) when compared with Sample 1-1-C that contained no blocked thiol compound.

TABLE IV shows the  $c \log P$  and N values for samples of TABLE III. Inventive samples have a  $c \log P$  values greater than 2.0 and N values greater than 6.5. In comparison, Comparative compound C-1 shows no improvement in Desktop Print Stability. It has an N value of 6, which is lower than the required minimum value of 6.5. Comparative compound C-2 is identical to inventive Compound PS-1 except that the sulfur has been replaced with an oxygen atom. This replacement results in a material providing no improvement in Desktop Print Stability. Comparative compound C-3 also shows no improvement in Desktop Print Stability. It has a  $c \log P$  value of -0.08, which is lower than the required minimum value of 2.0.

TABLE IV

| Sample | Compound | Inventive (I) or Comparative (C) | $c \log P$ | N Value |
|--------|----------|----------------------------------|------------|---------|
| 1-1-C  | None     | —                                | —          | —       |
| 1-2-C  | C-1      | Comparative                      | 7.88       | 6       |
| 1-3-C  | C-2      | Comparative                      | 10.10      | —       |
| 1-4-C  | C-3      | Comparative                      | -0.08      | 8       |
| 1-5-I  | PS-1     | Inventive                        | 10.5       | 19      |
| 1-6-I  | PS-2     | Inventive                        | 10.04      | 23      |
| 1-7-I  | PS-3     | Inventive                        | 19         | 19      |
| 1-8-I  | PS-4     | Inventive                        | 11.14      | 19      |
| 1-9-I  | PS-5     | Inventive                        | 11.14      | 19      |
| 1-10-I | PS-6     | Inventive                        | 9.51       | 17      |
| 1-11-I | PS-7     | Inventive                        | 7.99       | 21      |
| 1-12-I | PS-8     | Inventive                        | 8.56       | 23      |
| 1-13-I | PS-9     | Inventive                        | 10.17      | 19      |
| 1-14-I | PS-10    | Inventive                        | 7.55       | 13      |
| 1-15-I | PS-11    | Inventive                        | 5.59       | 9       |
| 1-16-I | PS-12    | Inventive                        | 3.56       | 13      |
| 1-17-I | PS-13    | Inventive                        | 5.76       | 12      |
| 1-18-I | PS-14    | Inventive                        | 3.12       | 11      |
| 20     | 1-19-I   | PS-15                            | 4.27       | 14      |
| 1-20-I | PS-16    | Inventive                        | 8.31       | 11      |
| 1-21-I | PS-17    | Inventive                        | 2.98       | 13      |
| 1-22-I | PS-20    | Inventive                        | 3.01       | 12      |
| 1-23-I | PS-22    | Inventive                        | 10.19      | 19      |
| 1-24-I | PS-23    | Inventive                        | 5.82       | 15      |
| 1-25-I | PS-25    | Inventive                        | 4.3        | 13      |
| 1-26-I | PS-30    | Inventive                        | 2.64       | 13      |
| 1-27-I | PS-31    | Inventive                        | 3.86       | 8       |

30

## EXAMPLE 2

## Evaluation of Blocked Aliphatic Thiol Compounds:

Components A, B, D, and F: Components A, B, D, and F were prepared as described in Example 1.

Component C: A mixture of 1,3-dimethylurea, succinimide, and xylitol was dissolved in water by heating at 50° C.

TABLE III

| Sample | Compound | Inventive or Comparative | Coating Weight [g/m <sup>2</sup> ] | $D_{min}$ | $D_{max}$ | Relative Speed-2 | 70/80 Desktop Print Stability [ $\Delta D_{min}$ ] |
|--------|----------|--------------------------|------------------------------------|-----------|-----------|------------------|----------------------------------------------------|
| 1-1-C  | None     | Comparative              | 0                                  | 0.325     | 2.91      | 100              | 0.51                                               |
| 1-2-C  | C-1      | Comparative              | 0.015                              | 0.292     | 2.24      | 91               | 0.56                                               |
| 1-3-C  | C-2      | Comparative              | 0.006                              | 0.336     | 3.05      | 102              | 0.52                                               |
| 1-4-C  | C-3      | Comparative              | 0.034                              | 0.321     | 2.86      | 97               | 0.48                                               |
| 1-5-I  | PS-1     | Inventive                | 0.031                              | 0.315     | 2.64      | 100              | 0.02                                               |
| 1-6-I  | PS-2     | Inventive                | 0.018                              | 0.315     | 2.73      | 100              | 0.02                                               |
| 1-7-I  | PS-3     | Inventive                | 0.028                              | 0.317     | 2.71      | 100              | 0.02                                               |
| 1-8-I  | PS-4     | Inventive                | 0.020                              | 0.323     | 2.65      | 101              | 0.01                                               |
| 1-9-I  | PS-5     | Inventive                | 0.019                              | 0.315     | 2.71      | 99               | 0.02                                               |
| 1-10-I | PS-6     | Inventive                | 0.026                              | 0.321     | 2.59      | 100              | 0.02                                               |
| 1-11-I | PS-7     | Inventive                | 0.030                              | 0.349     | 2.87      | 102              | 0.03                                               |
| 1-12-I | PS-8     | Inventive                | 0.037                              | 0.336     | 2.75      | 101              | 0.03                                               |
| 1-13-I | PS-9     | Inventive                | 0.027                              | 0.321     | 2.49      | 98               | 0.06                                               |
| 1-14-I | PS-10    | Inventive                | 0.015                              | 0.305     | 2.71      | 98               | 0.10                                               |
| 1-15-I | PS-11    | Inventive                | 0.015                              | 0.315     | 2.80      | 100              | 0.10                                               |
| 1-16-I | PS-12    | Inventive                | 0.058                              | 0.325     | 2.30      | 97               | 0.10                                               |
| 1-17-I | PS-13    | Inventive                | 0.047                              | 0.314     | 2.24      | 95               | 0.10                                               |
| 1-18-I | PS-14    | Inventive                | 0.030                              | 0.321     | 2.49      | 99               | 0.10                                               |
| 1-19-I | PS-15    | Inventive                | 0.065                              | 0.342     | 2.88      | 99               | 0.11                                               |
| 1-20-I | PS-16    | Inventive                | 0.028                              | 0.337     | 2.65      | 100              | 0.13                                               |
| 1-21-I | PS-17    | Inventive                | 0.062                              | 0.337     | 2.63      | 100              | 0.14                                               |
| 1-22-I | PS-20    | Inventive                | 0.057                              | 0.344     | 2.58      | 100              | 0.17                                               |
| 1-23-I | PS-22    | Inventive                | 0.027                              | 0.331     | 2.77      | 99               | 0.27                                               |
| 1-24-I | PS-23    | Inventive                | 0.057                              | 0.370     | 2.65      | 98               | 0.27                                               |
| 1-25-I | PS-25    | Inventive                | 0.028                              | 0.371     | 2.82      | 101              | 0.29                                               |
| 1-26-I | PS-30    | Inventive                | 0.022                              | 0.317     | 2.42      | 96               | 0.45                                               |
| 1-27-I | PS-31    | Inventive                | 0.023                              | 0.340     | 2.89      | 100              | 0.45                                               |

The dispersion of Developer D-1 described above was added to the above solution at room temperature.

Component E: A portion of hydrated gelatin (23% de-ionized lime-processed gelatin/77% water) was placed in a beaker and heated to 40° C. for 10 minutes. A portion of a dispersion of 6.5  $\mu$ m polystyrene beads in gelatin was placed in another beaker and heated to 40° C. for 10 minutes to melt. The gelatin melts were combined and to the mixture was added a 20% aqueous solution of 1,3-dimethylurea, a 5% aqueous solution of boric acid, and a 4% active aqueous solution of ZONYL® FS-300 surfactant.

Coating and Evaluation of Photothermographic Materials:

The components were coated and dried as described in Example 1 to give the imaging layer the dry composition shown below in TABLE V. The resulting photothermographic films were imaged using a sensitometer equipped with filters to provide an exposure simulating a phosphor emitting at 390 to 395 nm. Exposure was for  $\frac{1}{10}$  second using a 3000° K tungsten lamp. The films were developed and evaluated in a manner similar to that described in Example 1.

The results, shown below in TABLE VI demonstrate that the compounds of the present invention provide improved Desktop Print Stability while maintaining the sensitometry of the photothermographic films.

The results, shown below in TABLE VII, demonstrate that the  $c \log P$  and N values for the blocked thiol compounds are greater than 2.0 and 6.5 respectively.

TABLE V

| Component                       | Compound                          | Dry Coating Weight [g/m <sup>2</sup> ] |
|---------------------------------|-----------------------------------|----------------------------------------|
| <u>Photothermographic Layer</u> |                                   |                                        |
| A                               | Silver (from AgBZT/AgT-1)         | 1.40                                   |
| A                               | Lime processed gelatin            | 2.15                                   |
| A                               | 3-Methylbenzothiazolium Iodide    | 0.071                                  |
| A                               | Sodium benzotriazole              | 0.084                                  |
| A                               | Compound A-2                      | 0.072                                  |
| A                               | ZONYL® FS-300 surfactant          | 0.020                                  |
| B                               | Silver (from AgBrI emulsion)      | 0.25                                   |
| C                               | Succinimide                       | 0.17                                   |
| C                               | 1,3-Dimethylurea                  | 0.28                                   |
| C                               | Xylitol                           | 0.43                                   |
| C                               | Compound D-1                      | 3.64                                   |
| D                               | Blocked Aliphatic Thiol Compound  | See TABLE VI                           |
| <u>Overcoat Layer</u>           |                                   |                                        |
| E                               | De-ionized lime-processed gelatin | 1.40                                   |
| E                               | Boric acid                        | 0.046                                  |
| E                               | 1,3-Dimethylurea                  | 0.19                                   |
| E                               | ZONYL® FS-300 surfactant          | 0.070                                  |
| E                               | Matte bead S100                   | 0.094                                  |
| F                               | Compound VS-1                     | 0.083                                  |

TABLE VII

| Sample | Compound | Inventive (I) or Comparative (C) | c log P | N Value |
|--------|----------|----------------------------------|---------|---------|
| 2-1-C  | None     | Comparative                      | —       | —       |
| 2-2-I  | PS-1     | Inventive                        | 10.5    | 19      |
| 2-3-I  | PS-33    | Inventive                        | 17.72   | 19      |
| 2-4-I  | PS-35    | Inventive                        | 10.26   | 19      |
| 2-5-I  | PS-32    | Inventive                        | 10.77   | 19      |
| 2-6-I  | PS-34    | Inventive                        | 18.45   | 19      |
| 2-7-I  | PS-36    | Inventive                        | 12.23   | 19      |

## EXAMPLE 3

Photothermographic Materials Incorporating Blocked Aliphatic Thiol Compounds in the Presence or Absence of Boric Acid:

Components A, B, C, D, E, and F: Components A, B, C, D, E, and F were prepared as described in Example 2.

Coating and Evaluation of Photothermographic Materials:

The components were coated and dried as described in Example 1. The imaging layer and overcoat layer had the dry coating weights shown in TABLE VIII.

Samples were imaged, developed, and evaluated as described in Example 2. The results, shown below in TABLE IX, demonstrate the exceptional, unexpected, and synergistic ability of boric acid along with a blocked thiol compound to improve Desktop Print Stability. Sample 3-2-C incorporating only boric acid did not improve Desktop Print Stability. Sample 3-3-I incorporating only Compound PS-1 improved Desktop Print Stability (decreased  $\Delta D_{min}$  from 0.48 to 0.32, a  $[\Delta(\Delta D_{min})]$  of 0.16). Sample 3-4-I, incorporating both a blocked thiol and boric acid dramatically improved Desktop Print Stability, in that  $\Delta D_{min}$  decreased from 0.48 to 0.08 [a  $\Delta(\Delta D_{min})$  of 0.40].

TABLE VIII

| Component                       | Compound                  | Dry Coating Weight (g/m <sup>2</sup> ) |
|---------------------------------|---------------------------|----------------------------------------|
| <u>Photothermographic Layer</u> |                           |                                        |
| A                               | Silver (from AgBZT/AgT-1) | 1.40                                   |
| A                               | Lime processed gelatin    | 2.15                                   |

TABLE VI

| Sample | Compound | Inventive or Comparative | Coating Weight [g/m <sup>2</sup> ] | $D_{min}$ | $D_{max}$ | Relative Speed-2 | 70/80 Desktop Print Stability [ $\Delta D_{min}$ ] |
|--------|----------|--------------------------|------------------------------------|-----------|-----------|------------------|----------------------------------------------------|
| 2-1-C  | None     | Comparative              | 0                                  | 0.324     | 2.87      | 100              | 0.53                                               |
| 2-2-I  | PS-1     | Inventive                | 0.028                              | 0.327     | 2.80      | 102              | 0.05                                               |
| 2-3-I  | PS-33    | Inventive                | 0.063                              | 0.324     | 2.65      | 98               | 0.04                                               |
| 2-4-I  | PS-35    | Inventive                | 0.055                              | 0.333     | 2.59      | 102              | 0.05                                               |
| 2-5-I  | PS-32    | Inventive                | 0.063                              | 0.335     | 2.21      | 100              | 0.06                                               |
| 2-6-I  | PS-34    | Inventive                | 0.028                              | 0.325     | 2.86      | 101              | 0.09                                               |
| 2-7-I  | PS-36    | Inventive                | 0.070                              | 0.353     | 3.00      | 104              | 0.05                                               |

TABLE VIII-continued

| Component | Compound                          | Dry Coating Weight (g/m <sup>2</sup> ) | 5  |
|-----------|-----------------------------------|----------------------------------------|----|
| A         | 3-Methylbenzothiazolium Iodide    | 0.071                                  |    |
| A         | Sodium benzotriazole              | 0.084                                  |    |
| A         | Compound A-2                      | 0.072                                  |    |
| A         | ZONYL ® FS-300 surfactant         | 0.020                                  |    |
| B         | Silver (from AgBrI emulsion)      | 0.25                                   |    |
| C         | Succinimide                       | 0.17                                   | 10 |
| C         | 1,3-Dimethylurea                  | 0.28                                   |    |
| C         | Xylitol                           | 0.43                                   |    |
| C         | Compound D-1                      | 3.64                                   |    |
| D         | Compound PS-1                     | See TABLE IX                           |    |
|           |                                   | <u>Overcoat Layer</u>                  |    |
| E         | De-ionized lime-processed gelatin | 1.40                                   | 15 |
| E         | Boric acid                        | See TABLE IX                           |    |
| E         | 1,3-Dimethylurea                  | 0.10                                   |    |
| E         | ZONYL ® FS-300 surfactant         | 0.070                                  |    |
| E         | Matte bead S100                   | 0.094                                  |    |
| F         | Compound VS-1                     | 0.083                                  | 20 |

TABLE X

| Component                       | Compound                       | Dry Coating Weight [g/m <sup>2</sup> ] |
|---------------------------------|--------------------------------|----------------------------------------|
| <u>Photothermographic Layer</u> |                                |                                        |
| A                               | Silver (from AgBZT/AgT-1)      | 1.49                                   |
| A                               | Lime processed gelatin         | 2.28                                   |
| A                               | 3-Methylbenzothiazolium Iodide | 0.075                                  |
| A                               | Sodium benzotriazole           | 0.089                                  |
| A                               | Compound A-2                   | 0.076                                  |
| A                               | ZONYL ® FS-300 surfactant      | 0.022                                  |
| B                               | Silver (from AgBrI emulsion)   | 0.26                                   |
| C                               | Succinimide                    | 0.18                                   |
| C                               | 1,3-Dimethylurea               | 0.30                                   |
| C                               | Xylitol                        | 0.46                                   |
| C                               | Compound D-1                   | 3.86                                   |
| D                               | Blocked Thiol Compound         | See TABLE XI                           |

TABLE IX

| Sample | Inventive or Comparative | PS-1 [g/m <sup>2</sup> ] | Boric Acid [g/m <sup>2</sup> ] | 70/80 Desktop Print Stability |                  |                  |
|--------|--------------------------|--------------------------|--------------------------------|-------------------------------|------------------|------------------|
|        |                          |                          |                                | $\Delta D_{min}$              | D <sub>min</sub> | D <sub>max</sub> |
| 3-1-C  | Comparative              | 0                        | 0                              | 0.48                          | 0.292            | 2.94             |
| 3-2-C  | Comparative              | 0                        | 0.046                          | 0.53                          | 0.294            | 2.84             |
| 3-3-I  | Inventive                | 0.028                    | 0                              | 0.32                          | 0.296            | 2.82             |
| 3-4-I  | Inventive                | 0.028                    | 0.046                          | 0.08                          | 0.288            | 2.52             |

EXAMPLE 4

TABLE X-continued

| Component             | Compound                          | Dry Coating Weight [g/m <sup>2</sup> ] |
|-----------------------|-----------------------------------|----------------------------------------|
| <u>Overcoat Layer</u> |                                   |                                        |
| E                     | De-ionized lime-processed gelatin | 1.40                                   |
| E                     | Boric acid                        | 0.046                                  |
| E                     | 1,3-Dimethylurea                  | 0.19                                   |
| E                     | ZONYL ® FS300 surfactant          | 0.070                                  |
| E                     | Matte bead S100                   | 0.094                                  |
| F                     | Compound VS-1                     | 0.083                                  |

## Evaluation of Blocked Aliphatic Thiol Compounds:

Samples were prepared to compare the blocked aliphatic thiol compounds of the present invention with Comparative Compound C-4, described as Compound 1 in U.S. Pat. No. 3,824,103 (Pierce et al.).

Components A, B, C, D, E, and F: Components A, B, C, D, E, and F were prepared as described in Example 2.

The components were coated and dried as described in Example 1. The imaging layer and overcoat layer had the dry composition shown in TABLE X.

TABLE XI

| Sample | Compound | Inventive or Comparative | Coating Weight [g/m <sup>2</sup> ] | Mole ratio of compound/AgX | D <sub>min</sub> | D <sub>max</sub> | Relative Speed-2 |
|--------|----------|--------------------------|------------------------------------|----------------------------|------------------|------------------|------------------|
| 4-1-C  | C-4      | Comparative              | 0.014                              | 0.03                       | 0.320            | 2.87             | 100              |
| 4-2-I  | PS-1     | Inventive                | 0.030                              | 0.03                       | 0.313            | 2.62             | 100              |

Samples were imaged, developed, and evaluated as described in Example 2. The results are shown below in TABLES XI and XII.

Inventive Sample 4-2-I provided excellent Desktop Print Stability as evidenced by its  $\Delta D_{min}$  of 0.02. In contrast, Comparative Sample 4-1-C, which contained Comparative Compound C-4 at the same mole ratio relative to silver halide, had a  $\Delta D_{min}$  of 0.40.

TABLE XII

| Sample | Compound | Inventive or Comparative | 70/80 Desktop Print Stability [ $\Delta D_{min}$ ] |
|--------|----------|--------------------------|----------------------------------------------------|
| 4-1-C  | C-4      | Comparative              | 0.40                                               |
| 4-2-I  | PS-1     | Inventive                | 0.02                                               |

The invention has been described in detail with particular reference to certain preferred embodiments thereof, but it will be understood that variations and modifications can be effected within the spirit and scope of the invention.

What is claimed is:

1. A black-and-white photothermographic material comprising a support and having thereon at least one photothermographic imaging layer comprising a polymer binder and in reactive association:

- a. a photosensitive silver halide,
- b. a non-photosensitive source of reducible silver ions,
- c. a reducing agent for said reducible silver ions, and
- d. at least 1 mg/m<sup>2</sup> of a blocked aliphatic thiol compound that has a calculated octanol-water partition coefficient (clog P value) of 2.0 or greater, and an N value equal to or greater than 6.5.

2. The material of claim 1 wherein said blocked aliphatic thiol compound has a c log P value of 5 or greater, and an N value greater than 12.

3. The material of claim 2 wherein said blocked aliphatic thiol compound is represented by the following Structure (I) or (II):



wherein BLOCK-1 is a monovalent thermally releasing blocking group, BLOCK-2 is a multivalent thermally releasing blocking group, R<sub>1</sub> is a substituted or unsubstituted mono- or multivalent aliphatic group, m is an integer from 2 to 4, and n is integer of 1 to 4.

4. The material of claim 3 wherein BLOCK-1 is represented by one of the following Structures (III), (IV), (V), and (VI) and BLOCK-2 is represented by one of the following Structures (VII) and (VIII):



wherein R<sub>2</sub> is hydrogen, a substituted or unsubstituted aliphatic, heterocyclic, or (hetero)aromatic group, a R<sub>3</sub>SO<sub>2</sub>— group, or a R<sub>3</sub>—(C=O)— group, wherein R<sub>3</sub> is a substituted or unsubstituted aliphatic, heterocyclic, or (hetero) aromatic group, R<sub>4</sub>, R<sub>5</sub>, and R<sub>6</sub> are the same or different and are hydrogen or a substituted or unsubstituted aliphatic, heterocyclic, or (hetero)aromatic group, R<sub>7</sub> is a substituted or unsubstituted tertiary alkyl or tertiary aralkyl group, X<sub>2</sub> is R<sub>2</sub>—, HO—, H<sub>2</sub>N—, R<sub>2</sub>O—, R<sub>2</sub>S—, R<sub>2</sub>NH—, or R<sub>2</sub>R<sub>3</sub>N—, X<sub>1</sub> is oxygen or sulfur, R<sub>8</sub> is a multivalent substituted or unsubstituted aliphatic, heterocyclic, or (hetero)aromatic group, Y<sup>—</sup> is an anion sufficient to neutralize the positive charge, and\*designates the point of attachment of the thermally releasing blocking group to the sulfur of the thiol, with the proviso that any of R<sub>2</sub>, R<sub>3</sub>, R<sub>4</sub>, R<sub>5</sub>, R<sub>6</sub>, and X<sub>2</sub> may be linked to one another to form a (polycyclic)ring.

5. The material of claim 3 wherein R<sub>1</sub> is a substituted or 20 unsubstituted alkyl group having 10 to 24 carbon atoms, R<sub>9</sub>O<sub>2</sub>CCH<sub>2</sub>—, R<sub>9</sub>O<sub>2</sub>CCH<sub>2</sub>CH<sub>2</sub>—, R<sub>9</sub>NHC(=O)CH<sub>2</sub>CH<sub>2</sub>—, R<sub>9</sub>CONHCH<sub>2</sub>CH<sub>2</sub>—, R<sub>9</sub>SO<sub>2</sub>NHCH<sub>2</sub>CH<sub>2</sub>—, alkyl benzyl groups, R<sub>9</sub>NHCO<sub>2</sub>CH<sub>2</sub>CH<sub>2</sub>, or R<sub>9</sub>O<sub>2</sub>C(=O)NHCH<sub>2</sub>CH<sub>2</sub>— group, 25 wherein R<sub>9</sub> is an alkyl or aryl group having 6 or more carbon atoms.

6. The material of claim 1 wherein said blocked aliphatic thiol compound is present in an amount of from about 5 30 mg/m<sup>2</sup> to about 500 mg/m<sup>2</sup>.

7. The material of claim 1 wherein said blocked aliphatic thiol compound is one or more of the following Compounds PS-1 through PS-47:



49

-continued



50

-continued



**51**

-continued

**52**

-continued



-continued

(PS-47)



10

8. The material of claim 1 wherein said non-photosensitive source of reducible silver ions comprises a silver salt of a nitrogen-containing heterocyclic compound containing an imino group, said reducing agent is an ascorbic acid derivative, and said binder is gelatin, a gelatin derivative, or a poly(vinyl alcohol).  
15

9. The material of claim 1 further comprising a boron compound represented by Structure (IX):  
20



wherein X and Z are independently hydroxy, alkoxy, alkyl, acyl, or aryl groups, L is hydrogen, alkyl, aryl, or heteroaryl, or X and Z together represent carbon or heteroatoms sufficient to provide a heterocyclic ring with the boron atom, or still again, X, L, and Z together represent carbon or heteroatoms sufficient to provide a heterocyclic ring with the boron atom.  
25

10. The material of claim 1 wherein said photosensitive silver halide comprises tabular grains of silver bromide or silver bromoiodide, and further comprising a silver salt of a mercaptotriazole.  
30

11. The material of claim 1 wherein said non-photosensitive source of reducible silver ions comprises a first organic silver salt comprising a silver salt of a benzotriazole, and a second organic silver salt of a mercaptotriazole that is the following Compound (T-1):  
35



(T-1) 40

45

12. An imaging assembly comprising the photothermographic material of claim 1 that is arranged in association with one or more phosphor intensifying screens.  
50

13. The imaging assembly of claim 12 wherein said photothermographic material comprises a photosensitive silver halide that is spectrally sensitive to a wavelength of from about 300 to about 450 nm, and said phosphor intensifying screens are capable of emitting radiation in the range of from about 300 to about 450 nm.  
55

14. A method of forming a visible image comprising:  
60

- imagewise exposing the photothermographic material of claim 1 to form a latent image,
- simultaneously or sequentially, heating said exposed photothermographic material to develop said latent image into a visible image.  
65

15. The method of claim 14 wherein said imagewise exposing is carried out using visible or X-radiation.  
65

16. The method of claim 14 wherein said photothermographic material is arranged in association with one or more phosphor intensifying screens during imaging.

17. A black-and-white photothermographic material comprising a support and having thereon at least one photothermographic imaging layer comprising a hydrophilic polymer binder or a water-dispersible polymer latex binder and in reactive association:

- a photosensitive silver halide present as ultrathin tabular grains,
- a non-photosensitive source of reducible silver ions that comprises an organic silver salt comprising a silver salt of a nitrogen-containing heterocyclic compound containing an imino group,
- a reducing agent for said reducible silver ions that is an ascorbic acid derivative,
- a blocked aliphatic thiol compound that is one or more compounds of Structures PS-1 through PS-47, said blocked aliphatic thiol compound being present in an amount of from about 5 mg/m<sup>2</sup> to about 500 mg/m<sup>2</sup>, and
- boric acid or a boric acid ester compound,

wherein the compounds of Structures PS-1 through PS-47 are:



(PS-1)



(PS-2)



(PS-3)



(PS-4)



(PS-5)



(PS-6)



(PS-7)

**55**

-continued



(PS-14)



(PS-15)



50



(PS-16)



65

**56**

-continued

(PS-8)



(PS-18)



(PS-19)



(PS-20)



(PS-21)



(PS-22)



(PS-23)



(PS-24)



(PS-25)



(PS-26)



57

-continued



18. A black-and-white photothermographic material comprising a support having on a frontside thereof,

59

- a) one or more frontside photothermographic imaging layers comprising a hydrophilic polymer binder or a water-dispersible polymer latex binder, and in reactive association, a photosensitive silver halide, a non-photosensitive source of reducible silver ions, and a reducing agent for said non-photosensitive source reducible silver ions,
- b) said material comprising on the backside of said support, one or more backside photothermographic imaging layers having the same or different composition as said frontside photothermographic imaging layers, and
- c) optionally, an outermost protective layer disposed over said one or more photothermographic imaging layers on either or both sides of said support, wherein said material comprises one or more of the same or different blocked aliphatic thiol compounds on both sides of said support, each of said blocked aliphatic thiol compounds being present in the same or different amount of at least 1 mg/m<sup>2</sup> on both sides of said support, said blocked aliphatic thiol com-

60

pound having a calculated octanol-water partition coefficient (clog P value) of 2.0 or greater, and an N value equal to or greater than 6.5.

19. The material of claim 18 comprising the same blocked aliphatic thiol compound(s) at the same amount on both sides of said support.

20. The material of claim 18 wherein said photosensitive silver halide is sensitive to electromagnetic radiation of from about 300 to about 850 nm.

21. The material of claim 18 wherein said photothermographic imaging layers on both sides of said support are essentially the same, said reducing agent is a fatty acid ester of ascorbic acid, said photosensitive silver halide is present as tabular grains of silver bromide or silver bromoiodide, said non-photosensitive source of reducible silver ions comprising silver benzotriazole, said blocked aliphatic thiol compound is present in an amount of from about 5 mg/m<sup>2</sup> to about 100 mg/m<sup>2</sup> and further comprising boric acid or a boric acid ester compound.

\* \* \* \* \*